



US006916599B2

(12) **United States Patent**  
Nariyuki

(10) **Patent No.:** **US 6,916,599 B2**  
(45) **Date of Patent:** **Jul. 12, 2005**

(54) **PHOTOTHERMOGRAPHIC MATERIAL**

(75) Inventor: **Fumito Nariyuki, Kanagawa (JP)**

(73) Assignee: **Fuji Photo Film Co., Ltd., Kanagawa (JP)**

(\*) Notice: Subject to any disclaimer, the term of this patent is extended or adjusted under 35 U.S.C. 154(b) by 50 days.

(21) Appl. No.: **10/419,153**

(22) Filed: **Apr. 21, 2003**

(65) **Prior Publication Data**

US 2003/0224299 A1 Dec. 4, 2003

(30) **Foreign Application Priority Data**

Apr. 24, 2002 (JP) ..... P.2002-122270

(51) **Int. Cl.**<sup>7</sup> ..... **G03C 1/498; G03C 1/34**

(52) **U.S. Cl.** ..... **430/350; 430/567; 430/607; 430/610; 430/613; 430/619; 430/965**

(58) **Field of Search** ..... **430/619, 567, 430/965, 350, 613, 610, 607**

(56) **References Cited**

**U.S. PATENT DOCUMENTS**

5,698,380 A \* 12/1997 Toya ..... 430/363  
6,143,488 A 11/2000 Uytterhoeven et al.  
6,770,428 B2 \* 8/2004 Maskasky et al. ..... 430/350

**FOREIGN PATENT DOCUMENTS**

EP 1096310 A2 \* 5/2001 ..... G03C1/498  
JP 60-143331 \* 12/1983 ..... G03C1/02

\* cited by examiner

*Primary Examiner*—Thorl Chea

(74) *Attorney, Agent, or Firm*—Sughrue Mion, PLLC

(57) **ABSTRACT**

A photothermographic material comprising: a support; and a photosensitive silver halide, a nonphotosensitive organic silver salt, a reducing agent and a binder, wherein the photosensitive silver halide comprises 90% by mole or more of a silver iodide and has a silver iodobromide structure having an average silver iodide content of 35% by mole or less in vicinity of a surface thereof.

**15 Claims, 1 Drawing Sheet**

*FIG. 1*



## PHOTOTHERMOGRAPHIC MATERIAL

## FIELD OF THE INVENTION

The present invention relates to a photothermographic material and a process for producing an image by using the material.

## BACKGROUND OF THE INVENTION

In recent years, reduction of amounts of treated wastewater is earnestly demanded in the field of medical services from the standpoint of environment protection and space saving. According thereto, techniques relating to such photosensitive thermal developing photographic materials for medical diagnosis and photographic techniques are required that can be efficiently exposed in a laser image setter or a laser imager to form a sharp black image having high resolution and sharpness. In these photosensitive thermal developing photographic materials, the use of a solvent series treating chemical reagent can be eliminated to provide customers with such a simple thermal developing system that does not impair environments.

While there are the similar demands in the ordinary image forming materials, a medical image has such characteristics that high image quality with excellent sharpness and graininess is demanded owing to minute depiction, and further, a cold tone image is preferred owing to easiness in diagnosis. Under the current circumstances, various kinds of general hardcopy systems utilizing pigments and dyes are commercially available, such as an ink-jet printer and electrophotography, but there is no system that is sufficient as an output system for a medical image.

A thermal image formation system utilizing an organic silver salt is described, for example, in the specifications of U.S. Pat. Nos. 3,152,904 and 3,457,075, and B. Shely, "Thermally Processed Silver Systems", *Imaging Processes and Materials*, Noblette 8th ed., edited by Sturge, V. Walworth and A. Shepp, p. 2 (1996).

In particular, a photothermographic material generally has a photosensitive layer containing a binder matrix having dispersed therein a photocatalyst in a catalytically active amount (such as a silver halide), a reducing agent, a reducible silver halide (such as an organic silver salt), and depending on necessity, a toning agent for controlling the tone of silver. The photothermographic material forms a black silver image through imagewise exposure and heating to a high temperature (such as 80° C. or more) to cause a redox reaction between the silver halide or the reducible silver salt (functioning as an oxidizing agent) and the reducing agent. The redox reaction is accelerated by the catalytic function of a latent image of a silver halide formed by exposure. Therefore, the black silver image is formed in the exposed region. As a medical image forming system utilizing a photothermographic material disclosed in a large number of literatures, such as U.S. Pat. No. 2,910,377 and JP-B-43-4924, Dry Imager FM-DP L has been released by Fuji Medical Systems Inc.

In the production of the thermal image forming system utilizing an organic silver salt, the photothermographic material is produced by two methods, i.e., a method of coating a coating composition containing a solution formed by dissolving a polymer of a main binder in an organic solvent, followed by drying, and a method of coating a coating composition containing polymer fine particles of a main binder as an aqueous dispersion, followed by drying. The production equipment for the later method is simple

since a recovering step of a solvent is not necessary, and thus the method is advantageous for mass production.

The thermal image forming system utilizing an organic silver salt has a severe problem in storage stability of an image after developing treatment, particularly deterioration of a printout upon irradiation with light, due to the absence of a fixing step. As a method for improving the printout, a method of utilizing AgI formed by converting an organic silver salt is disclosed in U.S. Pat. No. 6,143,488 and EP 0,922,995. However, the methods of converting an organic silver salt with iodine as disclosed herein cannot provide sufficient sensitivity to fail to build a practical system.

Other examples of sensitive materials utilizing AgI are disclosed in WO97/48014, WO97/48015, U.S. Pat. No. 6,165,705, JP-A-8-297345 and Japanese Patent No. 2,785,129, but they fail to attain the sufficient sensitivity/fogging level and cannot be applied to practical use. A method for utilizing a silver halide having a large silver iodide content is being demanded.

JP-A-2000-305213 discloses an image forming process and a photosensitive material utilizing blue to ultraviolet laser light as an exposure light source, but AgI is not used therein, and the sensitivity thereof is insufficient.

## SUMMARY OF THE INVENTION

As a result of earnest investigations made by the inventors for developing a method for utilizing a silver halide having a large silver iodide content, it has been found that a photosensitive material with high sensitivity and high image quality can be obtained by using AgI in a system using blue to ultraviolet laser light. However, an expected sensitivity cannot be obtained only with AgI, but there is such a problem of causing a large desensitization width with increase of the polyhalogen amount.

In view of the foregoing problem, an object of the invention is to provide a photothermographic material that uses a silver halide having a high silver iodide content, has high sensitivity, and exhibits a small desensitization width due to a polyhalogen amount, and to provide a process for forming an image using the material.

The object of the invention has been accomplished by the following photothermographic materials.

1. A photothermographic material containing a support having thereon at least a photosensitive silver halide, a nonphotosensitive organic silver salt, a reducing agent and a binder, the photosensitive silver halide having a total silver iodide content of 90% by mole or more and having a silver iodobromide structure having an average silver iodide content of 35% by mole or less in vicinity of a surface thereof.

2. A photo thermographic material described in the item 1, wherein the photothermographic material contains a compound represented by the following formula (1) on a surface of the support, on which the photosensitive silver halide is contained, in an amount of 0.2 mole or more per 1 mole of the photosensitive silver halide:

(1)



wherein R<sup>1</sup> and R<sup>2</sup> each independently represents a hydrogen atom or a group that can be substituted on a benzene ring.

3. A photothermographic material described in the item 1 or 2, wherein the photosensitive silver halide is formed under a state where the nonphotosensitive organic silver salt is not present.

4. A photothermographic material described in one of the items 1 to 3, wherein the photothermographic material contains a compound represented by the formula (1) on a surface of the support, on which the photosensitive silver halide is contained, in an amount of 0.5 mole or more per 1 mole of the photosensitive silver halide.

5. A process for forming an image containing a step of exposing a photothermographic material described in one of the items 1 to 4 by using a laser light source having a light emission peak at a wavelength of from 350 to 450 nm.

6. A process for forming an image containing a step of exposing a photothermographic material described in one of the items 1 to 4 by using a laser light source having a light emission peak at a wavelength of from 390 to 430 nm.

7. A process for forming an image as described in the item 5 or 6, wherein the laser light has an exposure illuminance of 1 mW/mm<sup>2</sup> or more and an exposure time of 1 second or less.

It is important that the photosensitive silver halide used in the invention is a silver halide having a high silver iodide content having a total silver iodide content of 90% by mole or more and having a silver iodobromide structure having an average silver iodide content of 35% by mole or less in vicinity of a surface thereof.

It is preferred that the photosensitive silver halide used in the invention has, in at least part thereof, a phase absorbing light through direct transition. It has been well known in the art that a silver halide realizes absorption through direct transition at an exposure wavelength of from 350 to 450 nm with a high silver iodide structure having a hexagonal wurtzite structure or a cubic zincblende structure. However, a silver halide having a high silver iodide content is generally has low sensitivity and low utility value, and thus, the silver halide having the crystalline structure attaining the absorption through direct transition also generally has low sensitivity and low utility value in the field of photographic industry.

According to the studies made by the inventors, it has been found that in a photothermographic material containing a nonphotosensitive organic silver halide and a reducing agent, such a photosensitive material having a high silver iodide content attains high sensitivity and high sharpness by exposure of a large illuminance (1 mW/mm<sup>2</sup> or more) for a short period of time (1 second or less, preferably 10<sup>-2</sup> second or less, and more preferably 10<sup>-4</sup> second or less).

It has been also found that the photosensitive silver halide having a silver iodobromide structure in vicinity of a surface thereof can attain further high sensitivity while the image stability after processing is maintained, in comparison to those having no silver iodobromide structure.

According to the finding by the inventors, it is preferred that the size of the silver halide herein is 80 nm or less. The effect of the invention is particularly clearly exerted with a silver halide with a small particle size.

#### BRIEF DESCRIPTION OF THE DRAWING

##### [FIG. 1]

It is a diagram showing light absorption of a silver iodide emulsion that is preferably used in the invention.

#### DETAILED DESCRIPTION OF THE INVENTION

Elements constituting the photothermographic material of the invention will be described in detail below.

The photosensitive silver halide of the invention preferably has a total silver iodide content of 90% by mole or more. It is more preferred that the photosensitive silver halide has a total silver iodide content of from 95 to 98% by mole.

The silver halide of the invention preferably exhibits direct transition absorption ascribed to the silver iodide crystalline structure at a wavelength of from 350 to 450 nm. It can be conveniently discriminated as to whether or not a silver halide has light absorption through direct transition by observing exciton absorption ascribed to direct transition around a wavelength of from 400 to 430 nm.

FIG. 1 shows light absorption of a silver iodide emulsion that is preferably used in the invention. It is found that absorption ascribed to a high silver iodide exciton around 420 nm.

The direct transition light absorption high silver iodide phase may be present solely, but it is preferably present through junction with a silver halide exhibiting indirect transition in a wavelength range of from 350 to 450 nm, such as silver bromide, silver chloride, silver iodobromide, silver iodochloride and mixed crystals thereof.

The silver halide phase absorbing light through direct transition generally exhibits strong light absorption, but it has low sensitivity in comparison to an indirect transition silver halide phase exhibiting only weak absorption and has not been industrially utilized.

In the invention, preferred sensitivity can be obtained by exposing a high silver iodide photosensitive material having a silver iodobromide structure in vicinity of a surface thereof at an exposure wavelength of from 350 to 450 nm.

The wavelength for exposure is more preferably from 370 to 430 nm, further preferably from 390 to 430 nm, and particularly preferably from 390 to 420 nm.

The photosensitive silver halide of the invention exerts further preferred characteristics when it has a particle size of from 5 to 80 nm. The silver halide particles having the phase attaining direct transition absorption exhibits sufficient sensitivity when they have a small particle size of 80 nm or less.

The particle size of the photosensitive silver halide is more preferably from 5 to 60 nm, and further preferably from 10 to 50 nm. The particle size referred herein means a converted diameter of spheres having the same volume as the volume of the silver halide particles.

The formation process of a silver halide has been well known in the art, and for example, methods described in *Research Disclosure*, No. 17029 (June of 1978) and U.S. Pat. No. 3,700,458. Specifically, such a method can be used that a silver supplying compound and a halogen supplying compound are added to a solution of a polymer, such as gelatin, to prepare a photosensitive silver halide, which is then mixed with an organic silver salt. Methods described in paragraphs 0217 to 0224 of JP-A-11-119374, Japanese Patent Application No. Hei 11-98708 and JP-A-2000-347335 are also preferred.

Examples of the shape of the silver halide particles include cubic particles, octahedral particles, dodecahedral particles, tetradecahedral particles, tabular particles, spherical particles, columnar particles and irregular shape particles, and cubic particles are particularly preferred in the invention. Silver halide particles having rounded corners can also be preferably used.

65 The silver halide particles of the invention is characterized by having a silver iodobromide structure having an average silver iodide content of 35% by mole or less in the

vicinity of the surface. The average silver iodide content of the silver iodobromide structure in the vicinity of the surface is preferably 25% by mole or less, and more preferably 15% by mole or less.

In order to impart the silver iodobromide structure in the vicinity of the surface, a preparation method of core/shell particles can be employed, in which the interior of particles (core) is silver iodobromide, and the exterior thereof (shell) is silver bromide. A silver halide emulsion having a dual structure can be prepared with reference to JP-A-60-143331. In order to produce the high silver iodide particles having a silver iodobromide structure in the vicinity of the surface, such a method is employed in that a silver ion and a bromide ion are supplied in the form of a silver salt aqueous solution and a bromide aqueous solution to silver iodide host particles in a reactor. Silver bromide is grown as silver iodobromide while dissolving silver iodide to produce the silver iodobromide structure in the vicinity of the surface.

The vicinity of the surface referred in the invention means a region by a depth of about 5 nm from the surface. The composition of the region can be measured by such a surface analysis method as XPS (X-ray photoelectric spectroscopy) or ISS (ionic scattering spectroscopy).

The composition can also be confirmed by an X-ray diffraction method, and the average composition of the silver iodobromide structure and the ratio between the pure silver iodide part and the silver iodobromide part can also be measured.

In the invention, silver halide particles having a hexacyano metallic complex present on the outermost surface of the particles are preferred. Examples of the hexacyano metallic complex include  $[\text{Fe}(\text{CN})_6]^{4-}$ ,  $[\text{Fe}(\text{CN})_6]^{3-}$ ,  $[\text{Ru}(\text{CN})_6]^{3-}$ ,  $[\text{Os}(\text{CN})_6]^{4-}$ ,  $[\text{Co}(\text{CN})_6]^{3-}$ ,  $[\text{Rh}(\text{CN})_6]^{3-}$ ,  $[\text{Ir}(\text{CH})_6]^{3-}$ ,  $[\text{Cr}(\text{CN})_6]^{3-}$  and  $[\text{Re}(\text{CN})_6]^{3-}$ . In the invention a hexacyano Fe complex is preferred.

With respect to the hexacyano metallic complex, a counter anion is not important since it is present in the form of an ion in an aqueous solution, and it is preferably those suitable for a precipitation operation of a silver halide emulsion, such as an alkali metallic ion, e.g., a sodium ion, a potassium ion, a rubidium ion, a cesium ion and a lithium ion, an ammonium ion, and an alkylammonium ion (e.g., a tetramethylammonium ion, a tetraethylammonium ion, a tetrapropylammonium ion and a tetra(n-butyl)ammonium ion).

The hexacyano metallic complex may be added after mixing with a mixed solvent with a suitable organic solvent that can be mixed with water (such as an alcohol, an ether, a glycol, a ketone, an ester and an amide) or gelatin.

The addition amount of the hexacyano metallic complex is preferably from  $1 \times 10^{-5}$  to  $1 \times 10^{-2}$  mole, and more preferably from  $1 \times 10^{-4}$  to  $1 \times 10^{-3}$  mole, per 1 mole of silver.

In order to make the hexacyano metallic complex present on the outermost surface of the silver halide particles, the hexacyano metallic complex is directly added before completing the charging step, during the water washing step, during the dispersing step or before the chemical sensitizing step, which is after completing the addition of a silver nitrate aqueous solution used for forming the particles and before the chemical sensitizing step, in which chalcogen sensitization, such as sulfur sensitization, selenium sensitization and tellurium sensitization, or a noble metal sensitization, such as gold sensitization, is carried out. In order to prevent the silver halide particles from growing, it is preferred that the hexacyano metallic complex is added immediately after forming the particles, and it is also preferred that it is added before completing the charging step.

It is preferred that the addition of the hexacyano metallic complex is stated at the time when 96% by weight of the total amount of silver nitrate added for forming the particles has been added, more preferably at the time when 98% by weight thereof has been added, and particularly preferably at the time when 99% by weight thereof has been added.

When the hexacyano metallic complex is added immediately before completing the particle formation and after the addition of the silver nitrate aqueous solution, it can be adsorbed on the outermost surface of the silver halide particles, and almost all thereof forms a difficultly soluble salt with a silver ion on the surface of the particles. Because the silver salt of hexacyano iron(II) is more difficultly soluble than  $\text{AgI}$ , re-dissolution by fine particles can be prevented, and the silver halide fine particles of the invention having a small particle size can be produced.

The photosensitive silver halide particles of the invention may contain a metal or a metallic complex of Group 8 to Group 10 in the periodic table (showing from Group 1 to Group 18).

The metal or a central metal of the metallic complex of Group 8 to Group 10 is preferably rhodium, ruthenium and iridium. The metallic complex may be used solely, or two or more kinds of complexes of the same metal or different metals may be used in combination.

The content thereof is preferably in a range of from  $1 \times 10^{-9}$  to  $1 \times 10^{-3}$  mole per 1 mole of silver.

The heavy metal, the metallic complex and the method for adding them are described in JP-A-7-225449, paragraphs 0018 to 0024 of JP-A-11-65021 and paragraphs 0227 to 0240 of JP-A-11-119374.

A metallic atom that can be contained in the silver halide particles used in the invention (such as  $[\text{Fe}(\text{CH})_6]^{4-}$ ), a desalting method of the silver halide emulsion and a chemical sensitizing method are described in paragraphs 0046 to 0050 of JP-A-11-84574, paragraphs 0025 to 0031 of JP-A-11-65021 and paragraphs 0242 to 0250 of JP-A-11-119374.

As gelatin contained in the photosensitive silver halide emulsion used in the invention, various kinds of gelatin may be used. In order to maintain good dispersion conditions of the photosensitive silver halide emulsion in a coating composition containing an organic silver salt, low molecular weight gelatin having a molecular weight of from 500 to 60,000 is preferably used. The low molecular weight gelatin may be used upon forming the particles or upon dispersion after the desalting treatment, and it is used upon dispersion after the desalting treatment.

Various kinds of compounds that have been known as a chromatic sensitizer may be used in the invention to increase the inherent sensitivity. Examples of the compounds used in the invention include those disclosed in EP-A-587,338, U.S. Pat. Nos. 3,877,943 and 4,873,184, JP-A-5-341432, JP-A-11-109547 and JP-A-10-111543.

The photosensitive silver halide particles in the invention are preferably chemically sensitized by a sulfur sensitizing method, a selenium sensitizing method or a tellurium sensitizing method. Examples of the compound used in a sulfur sensitizing method, a selenium sensitizing method or a tellurium sensitizing method include the known compounds, such as those disclosed in JP-A-7-128768.

In particular, a tellurium sensitization is preferred in the invention, and the compounds disclosed in paragraph 0030 of JP-A-11-65021 and the compounds represented by the formulae (II), (III) and (IV) in JP-A-5-313284 are more preferred.

In the invention, the chemical sensitization may be carried out at any timing after forming the particles before coating, and examples of the timing include (1) before the spectral sensitization, (2) simultaneously with the spectral sensitization, (3) after the spectral sensitization and (4) immediately before coating. It is particularly preferably carried out after the spectral sensitization.

The using amount of a sulfur, selenium or tellurium sensitizer used in the invention is generally from  $10^{-8}$  to  $10^{-2}$  mole, and preferably from  $10^{-7}$  to  $10^{-3}$  mole, per mole of silver halide while it varies depending on the silver halide particles and the chemical aging conditions used. While the conditions of the chemical sensitization in the invention are not particularly limited, the pH may be from 5 to 8, the pAg may be from 6 to 11, and the temperature may be about from 40 to 95° C.

A thiosulfonic acid compound may be added to the silver halide emulsion used in the invention according to the method shown in EP-A-293,917.

The photosensitive silver halide emulsion in the photosensitive material used in the invention may be used solely, or two or more kinds thereof (for example, those having different average particle diameters, those having different halogen compositions, those having different crystal habits and those having different chemical sensitization conditions) may be used in combination. The gradation can be adjusted by using plural kinds of photosensitive silver halide having different sensitivities.

Examples of the techniques relating to these constitutions include those disclosed in JP-A-57-119341, JP-A-53-106125, JP-A-47-3929, JP-A-48-55730, JP-A-46-5187, JP-A-50-73627 and JP-A-57-150841. It is preferred that the emulsions have a difference in sensitivity of  $0.2 \log E$  among the emulsions.

The addition amount of the photosensitive silver halide in terms of a coated silver amount per  $1 \text{ m}^2$  of the photosensitive material is preferably from 0.03 to 0.6  $\text{g/m}^2$ , more preferably from 0.07 to 0.4  $\text{g/m}^2$ , and most preferably from 0.05 to 0.3  $\text{g/m}^2$ , and the addition amount of the photosensitive silver halide in terms of an amount per 1 mole of the organic silver salt is preferably from 0.01 to 0.3 mole, more preferably from 0.02 to 0.2 mole, and further preferably from 0.03 to 0.15 mole.

Examples of the mixing method and the mixing conditions of the photosensitive silver halide and the organic silver salt, which have been separately prepared, include such a method that the silver halide particles and the organic silver salt having been prepared are mixed, for example, in a high-speed agitator, a ball mill, a sand mill, a colloid mill, a vibration mill or a homogenizer, and such a method that the photosensitive silver halide having been prepared is mixed with the organic silver salt at certain timing during preparation, followed by completing the preparation of the organic silver salt.

As having been noted, it is preferred that the silver halide of the invention is preferably formed under a state where the organic silver salt is not present. Such a method is also preferred that two or more kinds of the organic silver salt aqueous dispersions and two or more kinds of the photosensitive silver salt aqueous dispersions are mixed from the standpoint of adjustment of the photographic characteristics.

The timing of adding the silver halide of the invention to a coating composition for forming an image forming layer is preferably 180 minutes before coating to immediately before coating, and more preferably 60 minutes before coating to 10 seconds before coating, but the mixing method and the

mixing conditions are not particularly limited as far as the effect of the invention is sufficiently exerted.

Specific examples of the mixing method include a method using a tank that designates a desired mean residence time calculated from the addition flow rate and the supplying rate to a coater, and a method using a static mixer disclosed in N. Harnby, M. F. Edwards and A. W. Nienow (translated by K. Takahashi), *Ekitai Kongo Gijutsu* (Liquid Mixing Techniques), Chapter 8, published by Nikkan Kogyo Shim bun Co., Ltd. (1989).

The gradation of the photosensitive material may be arbitrarily determined, and it is preferred that the average contrast in a density range of from 1.5 to 3.0 is from 1.5 to 10 for effective manifestation of the effect of the invention.

The average contrast referred herein means the gradient of a line passing an optical density of 1.5 and an optical density of 3.0 in a characteristic curve, in which the abscissa is logarithm of an exposure amount of laser, and the ordinate is an optical density of a photosensitive material after thermal development exposed at the exposure amount.

The average contrast is preferably from 1.5 to 10 for the improvement in performance of sharpness of characters. It is more preferably from 2.0 to 7, and further preferably from 2.5 to 6.

A toning agent used in the photothermographic material of the invention will be described.

The toning agent is described in paragraphs 0054 to 0055 of JP-A-10-62899, page, 21, lines 23 to 48 of EP 0,803764A1, JP-A-2000-356317 and Japanese Patent Application No. 2000-187298. Preferred examples thereof include a phthalazinone compound (such as phthalazinone and a phthalazinone derivative or a metallic salt thereof, e.g., 4-(1-naphthyl)phthalazinone, 6-chlorophthalazinone, 5,7-dimethoxyphthalazinone and 2,3-dihydro-1,4-phthalazindione); a combination of a phthalazinone compound and a phthalic acid compound (such as phthalic acid, 4-methylphthalic acid, 4-nitrophthalic acid, diammonium phthalate, sodium phthalate, potassium phthalate and tetrachlorophthalic anhydride); a phthalazine compound (such as phthalazine and a phthalazine derivative or a metallic salt thereof, e.g., 4-(1-naphthyl)phthalazine, 6-isopropylphthalazine, 6-t-butylphthalazine, 6-chlorophthalazine, 5,7-dimethoxyphthalazine and 2,3-dihydrophthalazine); and a combination of a phthalazine compound and a phthalic acid compound, and the combination of a phthalazine compound and a phthalic acid compound is particularly preferred.

As the toning agent of the invention, a compound represented by the formula (1) is preferred.

In the formula (1),  $R^1$  and  $R^2$  each independently represents a hydrogen atom or a group that can be substituted on a benzene ring.

Examples of the group that can be substituted on a benzene ring in  $R^1$  and  $R^2$  include an alkyl group, an aryl group, a halogen atom, a hydroxyl group and an alkoxy group. Specific examples of the group that can be substituted include a methyl group, an ethyl group, an isopropyl group, an isobutyl group, a t-butyl group, a chlorine atom, a methoxy group and a hydroxyl group.

Specific examples of the compound represented by the formula (1) include 6-isopropylphthalazine, 6-t-butylphthalazine, 5-chlorophthalazine, 5,7-dimethoxyphthalazine and 2,3-dihydrophthalazine, and 6-isopropylphthalazine is particularly preferred.

The addition amount of the toning agent in the invention is preferably 0.2 mole or more, more preferably 0.5 mole or

more, and further preferably 1 mole or more, per 1 mole of the photosensitive silver halide.

The toning agent is preferably a combination with a phthalic acid compound. Particularly preferred combinations include a combination of 6-isopropylphthalazine and phthalic acid or 4-methylphthalic acid.

The organic silver salt that can be used in the invention is such a silver salt that is relatively stable to light but forms a silver image upon heating to a temperature of 80° C. or more in the presence of an exposed photocatalyst (such as a latent image of a photosensitive silver halide) and a reducing agent. The organic silver salt may be an arbitrary organic substance containing a source capable of reducing a silver ion.

The nonphotosensitive organic silver salt is described in paragraphs 0048 to 0049 of JP-A-10-62899, page 18, line 24 to page 19, line 37 of EP 0.803,764A1, EP 0,962,812A1, JP-A-11-349591, JP-A-2000-7683 and JP-A-2000-72711.

The organic silver salt in the invention is preferably a silver salt of an organic acid, particularly a silver salt of a long chain aliphatic carboxylic acid (having from 10 to 30, preferably from 15 to 28, carbon atoms). Preferred examples of the aliphatic acid silver salt include silver behenate, silver arachidinate, silver stearate, silver oleate, silver laurate, silver caproate, silver myristate, silver palmitate and a mixture thereof.

Among these aliphatic acid silver salts, it is preferred in the invention to use an aliphatic acid silver salt having a content of silver behenate of 50% by mole or more, more preferably 80% by mole or more, and further preferably 90% by mole or more.

The shape of the organic silver salt that can be used in the invention is not particularly limited and may be an acicular shape, a rod shape, a tabular shape or a squamous shape.

An organic salt having a squamous shape is preferably used in the invention. An organic salt having a short acicular shape having a ratio of the major axis and the minor axis of 5 or less, a rectangular parallelepipedal shape, a cubic shape or an irregular shape is also preferably used. These organic silver salt particles have such characteristics that they suffer small fogging on thermal development in comparison to long acicular particles having a ratio of the major axis and the minor axis of 5 or more.

The organic silver salt having a squamous shape in the invention is defined as follows. The organic silver salt is observed with an electron microscope, and the shape of the organic silver salt particle is approximated as a rectangular parallelepiped. The edges of the rectangular parallelepiped is designated as a, b and c in the order from the shortest edges to the longest edges (in which c may be the same as b), and the value x is calculated from a and b according to the following equation.

$$x=b/a$$

The value x is obtained for about 200 particles, and the average value thereof is designated as x (average). The particles satisfying the condition  $x \text{ (average)} \geq 1.5$  are designated as those having a squamous shape. The value x (average) preferably satisfies the condition  $30 \geq x \text{ (average)} \geq 1.5$ , and more preferably  $20 \geq x \text{ (average)} \geq 2.0$ . The acicular shape is designated by the condition  $1.5 \geq x \text{ (average)} \geq 1$ .

In the squamous particles, the value a can be understood as a thickness of a tabular particle having a plane with edges b and c as a principal plane. The average value of a is preferably from 0.01 to 0.23  $\mu\text{m}$ , and more preferably from

0.1 to 0.20  $\mu\text{m}$ . The average value of c/b is preferably 1 to 6, more preferably from 1.05 to 4, further preferably from 1.1 to 3, and particularly preferably from 1.1 to 2.

The particle size distribution of the organic silver salt is preferably monodisperse. The term monodisperse herein means that a percentage of a value obtained by dividing the standard deviations of the minor axis and the major axis by the minor axis and the major axis, respectively, is 100% or less, more preferably 80% or less, and further preferably 50% or less. The shape of the organic silver salt can be measured from a transmission electron micrograph of the organic silver salt dispersion.

Another method for measuring the monodispersity includes a method of obtaining a standard deviation of the volume weighted average diameter of the organic silver salt, and the percentage of a value obtained by dividing by the volume weighted average diameter (variation coefficient) is preferably 100% or less, more preferably 80% or less, and further preferably 50% or less. The measurement method therefor includes such a method that the organic silver salt dispersed in a liquid is irradiated with laser light, and an autocorrelation function with respect to time of the fluctuation of the scattered light therefrom is measured to obtain the particle size (volume weighted average diameter).

The production method and the dispersion method of the organic silver salt used in the invention can be carried out according to the ordinary methods Examples thereof include those described in JP-A-10-62899, EP0,803,763A1, EP 0,962,812A1, JP-A-11-349591, JP-A-2000-7683, JP-A-2000-72711, JP-A-11-348228, JP-A-11-348229, JP-A-11-348230, JP-A-11-203413, and Japanese Patent Application Nos. 2000-90093, 2000-195621, 2000-191226, 2000-213813, 2000-214155 and 2000-191226.

In the case where the photosensitive silver salt is present upon dispersing the organic silver salt, the fogging is increased to lower the sensitivity in a considerable extent, and therefore, it is preferred that the photosensitive silver halide is substantially not contained upon dispersing.

The amount of the photosensitive silver salt in an aqueous dispersion to be dispersed is preferably 1% by mole or less per 1 mole of the silver halide in the dispersion, more preferably 0.1% by mole, and further preferably no positive addition of the photosensitive silver salt.

In the invention, the photosensitive material can be produced by mixing the organic silver salt aqueous dispersion and the photosensitive silver salt aqueous dispersion. The mixing ratio of the organic silver salt and the photosensitive silver salt may be selected depending on purposes, and the ratio of the photosensitive silver halide to the organic silver salt is preferably in a range of from 1 to 30% by mole, more preferably from 2 to 20% by mole, and particularly preferably from 3 to 15% by mole.

Such a method is also preferred that two or more kinds of the organic silver salt aqueous dispersions and two or more kinds of the photosensitive silver salt aqueous dispersions are mixed from the standpoint of adjustment of the photographic characteristics.

The organic silver salt of the invention can be used in a desired amount, and the amount thereof in terms of silver is preferably from 0.1 to 5  $\text{g}/\text{m}^2$ , more preferably from 0.3 to 3  $\text{g}/\text{m}^2$ , and further preferably from 0.5 to 2  $\text{g}/\text{m}^2$ .

The photothermographic material of the invention preferably contains a thermal developer as a reducing agent for the organic silver salt. The reducing agent for the organic silver salt may be an arbitrary substance (preferably an organic substance) capable of reducing a silver ion to metallic silver.

## 11

Examples of the reducing agent are disclosed in paragraphs 0043 to 0045 of JP-A-11-65021 and page 7, line 34 to page 18, line 12 of EP 0,803,764A1.

In the invention, the reducing agent is preferably a so-called hindered phenol reducing agent having a substituent at an ortho position of a phenolic hydroxyl group or a bisphenol reducing agent, and more preferably a compound represented by the following formula (R):



wherein R<sup>11</sup> and R<sup>11'</sup> each independently represents an alkyl group having from 1 to 20 carbon atoms; R<sup>12</sup> and R<sup>12'</sup> each independently represents a hydrogen atom or a group that can be substituted on a benzene ring; L represents an —S— group or a —CHR<sup>13</sup>— group; R<sup>13</sup> represents a hydrogen atom or an alkyl group having from 1 to 20 carbon atoms; X<sup>1</sup> and X<sup>1'</sup> each independently represents a hydrogen atom or a group that can be substituted on a benzene ring.

The formula (R) will be described in detail.

R<sup>11</sup> and R<sup>11'</sup> each independently represents a substituted or unsubstituted alkyl group having from 1 to 20 carbon atoms. The substituent on the alkyl group is not particularly limited, and preferred examples thereof include an aryl group, a hydroxyl group, an alkoxy group, an aryloxy group, an alkylthio group, an arylthio group, an acyl amino group, a sulfon amide group, a sulfonyl group, a phosphoryl group, an acyl group, a carbamoyl group, an ester group, a ureido group, a urethane group and a halogen atom.

R<sup>12</sup> and R<sup>12'</sup> each independently represents a hydrogen atom or a group that can be substituted on a benzene ring, and X<sup>1</sup> and X<sup>1'</sup> also each independently represents a hydrogen atom or a group that can be substituted on a benzene ring. Preferred examples of the group that can be substituted on a benzene ring include an alkyl group, an aryl group, a halogen atom, an alkoxy group and an acylamino group.

L represents an —S— group or a —CHR<sup>13</sup>— group. R<sup>13</sup> represents a hydrogen atom or an alkyl group having from 1 to 20 carbon atoms, and the alkyl group may have a substituent. Specific examples of the unsubstituted alkyl group represented by R<sup>13</sup> include a methyl group, an ethyl group, a propyl group, a butyl group, a heptyl group, an undecyl group, an isopropyl group, a 1-ethylpentyl group and a 2,4,4-trimethylpentyl group. Examples of the substituent on the alkyl group include those exemplified for the substituent of R<sup>11</sup>.

R<sup>11</sup> and R<sup>11'</sup> preferably represents a secondary or tertiary alkyl group having from 3 to 15 carbon atoms, and specific examples thereof include an isopropyl group, an isobutyl group, a t-butyl group, a t-amyl group, a t-octyl group, a cyclohexyl group, a cyclopentyl group, a 1-methylcyclohexyl group and a 1-methylcyclopropyl group.

R<sup>11</sup> and R<sup>11'</sup> more preferably represents a tertiary alkyl group having from 4 to 12 carbon atoms, and a t-butyl group, a t-amyl group and a 1-methylcyclohexyl group are further preferred among them with a t-butyl group being most preferred.

R<sup>12</sup> and R<sup>12'</sup> each preferably represents an alkyl group having from 1 to 20 carbon atoms, and specific examples

## 12

thereof include a methyl group, an ethyl group, a propyl group, a butyl group, an isopropyl group, a t-butyl group, a t-amyl group, a cyclohexyl group, a 1-methylcyclohexyl group, a benzyl group, a methoxymethyl group and a methoxyethyl group. More preferred examples thereof include a methyl group, an ethyl group, a propyl group, an isopropyl group and a t-butyl group.

X<sup>1</sup> and X<sup>1'</sup> each preferably represents a hydrogen atom, a halogen atom or an alkyl group, and more preferably represents a hydrogen atom.

L preferably represents a —CHR<sup>13</sup>— group.

R<sup>13</sup> preferably represents a hydrogen atom or an alkyl group having from 1 to 15 carbon atoms, and preferred examples of the alkyl group include a methyl group, an ethyl group, a propyl group, an isopropyl group and a 2,4,4-trimethylpentyl group. Particularly preferred examples of R<sup>13</sup> include a hydrogen atom, a methyl group, an ethyl group, a propyl group and an isopropyl group.

In the case where R<sup>13</sup> represents a hydrogen atom, R<sup>12</sup> and R<sup>12'</sup> each preferably represents an alkyl group having from 2 to 5 carbon atoms, more preferably an ethyl group or a propyl group, and most preferably an ethyl group.

In the case where R<sup>13</sup> represents a primary or secondary alkyl group having from 1 to 8 carbon atoms, R<sup>12</sup> and R<sup>12'</sup> each preferably represents a methyl group. Preferred examples of the primary or secondary alkyl group having from 1 to 8 carbon atoms of R<sup>13</sup> include a methyl group, an ethyl group, a propyl group and an isopropyl group, and a methyl group, an ethyl group and a propyl group are more preferred.

In the case where all R<sup>11</sup>, R<sup>11'</sup>, R<sup>12</sup> and R<sup>12'</sup> represent methyl groups, R<sup>13</sup> preferably represents a secondary alkyl group. Examples of the secondary alkyl group of R<sup>13</sup> in this case include an isopropyl group, an isobutyl group and a 1-ethylpentyl group, and an isopropyl group is more preferred.

The reducing agent varies in thermal developing property and developed silver tone depending on the combination of R<sup>11</sup>, R<sup>11'</sup>, R<sup>12</sup>, R<sup>12'</sup> and R<sup>13</sup>. The properties can be adjusted by combining two or more kinds of the reducing agents, and therefore, it is preferred that two or more kinds of the reducing agents are used in combination depending on purpose.

Specific examples of the reducing agent of the invention including the compounds represented by the formula (R) will be described below, but the invention is not construed as being limited thereto.

(I-1)



**13**  
-continued**14**  
-continued



17

-continued

(I-30)



(I-31)



(I-32)



(I-33)

30



(I-34)



The addition amount of the reducing agent in the invention is preferably from 0.1 to 3.0 g/m<sup>2</sup>, more preferably from 0.2 to 1.5 g/m<sup>2</sup>, and further preferably from 0.3 to 1.0 g/m<sup>2</sup>.

It is preferably contained in an amount of from 5 to 50% by mole per 1 mole of silver on the surface, on which the image forming layer is formed, more preferably from 8 to 30% by mole, and further preferably from 10 to 20% by mole. It is preferably contained in the image forming layer.

The reducing agent may be contained in a coating composition in any form and any method, e.g., in the form of a solution, an emulsion dispersion or a solid fine particle dispersion, to be contained in the photosensitive material.

Examples of the well-known method therefor include a method, in which it is dissolved by using an auxiliary solvent, such as an oil, e.g., dibutyl phthalate, tricresyl phosphate, glyceril triacetate and diethyl phthalate, ethyl acetate and cyclohexanone, and an emulsion dispersion is mechanically produced.

Examples of the solid fine particle dispersion method include such a method in that powder of the reducing agent

18

is dispersed in a suitable solvent, such as water, with a ball mill, a colloid mill, a vibration ball mill, a sand mill, a jet mill, a roller mill or ultrasonic wave, so as to form a solid dispersion. A protective colloid (such as polyvinyl alcohol) and a surface active agent (such as an anionic surface active agent, e.g., sodium triisopropylnaphthalenesulfonate (a mixture of isomers with different substitution positions of the three isopropyl groups)) may be used herein. Beads, such as zirconia, are generally used as a dispersing medium in the foregoing mills, and therefore, Zr or the like substance is eluted from the beads into the dispersion. The amount thereof is generally in a range of from 1 to 1,000 ppm while it depends on the dispersion conditions. There is no practical problem when the content of Zr in the photosensitive material is 0.5 mg or less per 1 g of silver.

It is preferred that an antiseptic agent (such as sodium benzoisothiazolinone) is added to the aqueous dispersion.

In the photothermographic of the invention, a development accelerating agent, such as a phosphonic amide phenol compound represented by the formula (A) in JP-A-2000-267222 and JP-A-2000-330234, a hindered phenol compound represented by the formula (II) in JP-A-2001-92075, a hydrazine compound represented by the formula (1) in JP-A-10-62895 and JP-A-11-15116, and a phenol or naphthol compound represented by the formula (2) in Japanese Patent Application No. 2000-76240, is preferably used.

The development accelerating agent is generally used in an amount in a range of from 0.1 to 20% by mole, preferably in a range of from 0.5 to 10% by mole, and more preferably in a range of from 1 to 5% by mole, based on the reducing agent. The introduction method therefor may be the similar method as used for the reducing agent, and it is particularly preferably added in the form of a solid dispersion or an emulsion dispersion.

In the case where it is added in the form of an emulsion dispersion, it is preferably added as an emulsion dispersion formed by dispersing by using a high boiling point solvent, which is in a solid state at ordinary temperature, and an auxiliary solvent having a low boiling point, or as a so-called oilless emulsion dispersion using no high boiling point solvent.

A hydrogen bonding compound used in the invention will be described.

In the case where the reducing agent contains an aromatic hydroxyl group (—OH), particularly in the case of the bisphenol compound, it is preferred that a non-reducing compound having a group capable of forming a hydrogen bond with that group is used in combination.

Examples of the group forming a hydrogen bond with a hydroxyl group or an amino group include a phosphoryl group, a sulfoxide group, a sulfonyl group, a carbonyl group, an amide group, an ester group, a urethane group, a ureido group, a tertiary amino group and a nitrogen-containing aromatic group.

Among these, compounds having a phosphoryl group, a sulfoxide group, an amide group (provided that it has no >N—H group but is blocked as >N—Ra (wherein Ra represents a substituent other than H)), a urethane group (provided that it has no >N—H group but is blocked as >N—Ra (wherein Ra represents a substituent other than H)), a ureido group (provided that it has no >N—H group but is blocked as >N—Ra (wherein Ra represents a substituent other than H)) are preferred.

The hydrogen bonding compound in the invention is particularly preferably a compound represented by the following formula (D):



wherein R<sup>21</sup> to R<sup>23</sup> each independently represents an alkyl group, an aryl group, an alkoxy group, an aryloxy group, an amino group or a heterocyclic group, which may be unsubstituted or substituted.

Examples of the substituent in the case where the groups represented by R<sup>21</sup> to R<sup>23</sup> are substituted include a halogen atom, an alkyl group, an aryl group, an alkoxy group, an amino group, an acyl group, an acylamino group, an alkylthio group, an arylthio group, a sulfonamide group, an acyloxy group, an oxycarbonyl group, a carbamoyl group, a sulfamoyl group, a sulfonyl group and a phosphoryl group. Preferred examples of the substituent include an alkyl group and an aryl group, and examples thereof include a methyl group, an ethyl group, an isopropyl group, a t-butyl group, a t-octyl group, a phenyl group, a 4-alkoxyphenyl group and a 4-acyloxyphenyl group.

Specific examples of the alkyl group represented by R<sup>21</sup> to R<sup>23</sup> include a methyl group, an ethyl group, a butyl group, an octyl group, a dodecyl group, an isopropyl group, a t-butyl group, a t-amyl group, a t-octyl group, a cyclohexyl group, a 1-methylcyclohexyl group, a benzyl group, a phenethyl group and a 2-phenoxypropyl group.

Examples of the aryl group include a phenyl group, a cresyl group, a xylyl group, a naphthyl group, a 4-t-butylphenyl group, a 4-t-octylphenyl group, a 4-anisidyl group and a 3,5-dichlorophenyl group.

Examples of the alkoxy group include a methoxy group, an ethoxy group, a butoxy group, an octyloxy group, a 2-ethylhexyloxy group, a 3,5,5-trimethylhexyloxy group, a dodecyloxy group, a cyclohexyloxy group, a 4-methylcyclohexyloxy group and a benzyloxy group.

Examples of the aryloxy group include a phenoxy group, a cresyloxy group, an isopropylphenoxy group, a 4-t-butylphenoxy group, a naphthoxy group and a biphenyloxy group.

Examples of the amino group include a dimethylamino group, a diethylamino group, a dibutylamino group, a diethylamino group, an N-methyl-N-hexylamino group, a dicyclohexylamino group, a diphenylamino group and an N-methyl-N-phenylamino group.

R<sup>21</sup> to R<sup>23</sup> each preferably represents an alkyl group, an aryl group, an alkoxy group or an aryloxy group. It is preferred from the standpoint of the effect of the invention that at least one of R<sup>21</sup> to R<sup>23</sup> represents an alkyl group or an aryl group, and it is more preferred that two or more of them each represents an alkyl group or an aryl group. A compound having the same groups for R<sup>21</sup> to R<sup>23</sup> is preferred since the compound can be inexpensively available.

Specific examples of the hydrogen bonding agent of the invention including the compounds represented by the formula (D) will be described below, but the invention is not construed as being limited thereto.



**21**

-continued

**22**

-continued



Specific examples of the hydrogen bonding compound include those disclosed in European Patent No. 1,096,310 and Japanese Patent Application Nos. 2000-270498 and 2001-124796, in addition to the foregoing compounds.

The compound represented by the formula (D) of the invention can be contained in a coating composition, as similar to the reducing agent, in the form of a solution, an emulsion dispersion or a solid dispersed fine particle dispersion to be used in the photosensitive material. The compound of the invention forms a hydrogen bonding complex with a compound having a phenolic hydroxyl group or an amino group in the form of a solution, and can be isolated in as a complex in the form of crystals depending on the combination of the reducing agent and the compound represented by the formula (D) of the invention. The use of the thus isolated crystalline powder as a solid dispersed fine particle dispersion is preferred for obtaining stable performance. Such a method is also preferably employed in that the reducing agent and the compound represented by the formula (D) of the invention are mixed in the form of powder and then subjected to complex formation upon dispersing by using a suitable dispersing agent with, for example, a sand grinder mill (SGM). The compound represented by the formula (D) is preferably used in an amount of from 1 to 200% by mole, more preferably from 10 to 150% by mole, and further preferably from 20 to 100% by mole, based on the reducing agent.

A binder used in the invention will be described.

The binder of the layer containing the organic silver salt of the invention may be any polymer, and suitable examples of the polymer include those that are transparent or translucent and are generally colorless. Examples thereof include a natural resin, a synthetic resin, polymer or copolymer, and other media that form a film, such as a gelatin compound, a rubber compound, a poly (vinyl alcohol) compound, a hydroxyethylcellulose compound, a cellulose acetate compound, a cellulose acetate butyrate compound, a poly (vinylpyrrolidone) compound, casein, starch, a poly(acrylic acid) compound, a poly(methyl methacrylate) compound, a poly (vinyl chloride) compound, a poly(methacrylic acid) compound, a styrene-maleic anhydride copolymer, a styrene-acrylonitrile copolymer, a styrene-butadiene copolymer, a poly(vinyl acetal) compound (for example, poly(vinyl formal) and poly(vinyl, butyral)), a poly(ester) compound, a poly(urethane) compound, a phenoxy resin, a poly(vinylidene chloride) compound, a poly(epoxide) compound, a poly(carbonate) compound, a poly(vinyl acetate) compound, a poly(olefin) compound, a cellulose ester compound and a poly(amide) compound.

The binder may be formed into a coated layer from a solution of water or an organic solvent or from an emulsion.

The binder that can be used in combination in the layer containing the organic silver salt in the invention preferably has a glass transition temperature  $T_g$  of from 0 to 80° C., more preferably from 10 to 70° C., and further preferably from 15 to 65° C. (hereinafter sometimes referred to as a high  $T_g$  binder).

$T_g$  in the invention is calculated according to the following equation.

$$1/T_g = \sum (X_i/T_{gi})$$

Herein, it is assumed that the polymer is formed by copolymerizing  $n$  monomers, i.e.,  $i=1$  to  $n$ .  $X_i$  means the weight fraction of the  $i$ -th monomer ( $\sum X_i=1$ ), and  $T_{gi}$  means the glass transition temperature (in terms of absolute temperature) of a homopolymer of the  $i$ -th monomer.  $\Sigma$  means the sum of from  $i=1$  to  $n$ .

For the values of the glass transition temperatures of the homopolymers of the respective monomers ( $T_{gi}$ ), the values disclosed in J. Brandrup and E. H. Immergut, *Polymer Handbook* 3rd Edition, published by Wiley-Interscience (1989).

Two or more kinds of binders may be used in combination depending on necessity. A binder having a glass transition temperature of 20° C. or more and that having a glass transition temperature of less than 20° C. may be used in combination. In the case where two or more kinds of polymers having different  $T_g$  values are used in combination, it is preferred that the weight average  $T_g$  falls within the foregoing range.

In the invention, a coated film of the layer containing the organic silver salt is preferably formed by coating and drying a coating composition containing water in an amount of 30% by weight or more based on the total amount of the solvent contained.

In the case where the layer containing the organic silver salt is formed by coating and drying a coating composition containing water in an amount of 30% by weight or more based on the total amount of the solvent contained, and in the case where the binder of the layer containing the organic silver salt can be dissolved or dispersed in an aqueous solvent (water solvent), the performance is improved when the binder is formed with polymer latex having an equilibrium water content at 25° C. and 60% RH of 2% by weight

or less. The most preferred embodiment is that having been prepared to have an ionic electroconductivity of 2.5 mS/cm or less, and examples of the preparation method therefor include a method of purifying the polymer after synthesis by using a separation functional membrane.

The aqueous solvent herein, in which the polymer can be dissolved or dispersed, means water or a mixture of water and 70% by weight or less of a water miscible organic solvent.

Examples of the water miscible organic solvent include an alcohol solvent, such as methyl alcohol, ethyl alcohol and propyl alcohol, a cellosolve solvent, such as methylcellosolve, ethylcellosolve and butylcellosolve, ethyl acetate, and dimethylformamide.

In the case where the polymer is not thermodynamically dissolved in a system but is present in a dispersed state, the system is referred by the term aqueous solvent herein.

The term "equilibrium water content at 25° C. and 60% RH (% by weight)" herein can be expressed by using the weight  $W_1$  of the polymer that is in a humidity equilibrium under an atmosphere at 25° C. and 60% RH and the weight  $W_0$  of the polymer that is in an absolute dry state according to the following equation.

$$\text{Equilibrium water content at 25° C. and 60% RH} = \frac{(W_1 - W_0)}{W_0} \times 100$$

With respect to the definition of the water content and the measurement method therefor, for example, *Kobunshi Jikken Koza 14* (Polymer Experimental Course 14), *Kobunshi Zairyo Shiken-ho* (Test Methods of Polymer Materials), edited by Polymer Society of Japan, published by Chijin Shokan Co., Ltd. can be referred.

The equilibrium water content at 25° C. and 60% RH of the polymer of the binder of the invention is preferably 2% by weight or less, more preferably from 0.01 to 1.5% by weight, and further preferably from 0.02 to 1% by weight.

In the invention, a polymer that can be dispersed in an aqueous solvent is particularly preferred. Examples of the dispersed state include latex having fine particles of a water insoluble hydrophobic polymer dispersed therein and a dispersed state having a polymer dispersed therein by forming a molecular state or a micellar state, and the particles dispersed in a latex state are more preferred.

The dispersed particles generally have an average particle diameter of from 1 to 50,000 nm, preferably from 5 to 1,000 nm, more preferably from 10 to 500 nm, and further preferably from 50 to 200 nm. The particle size distribution of the dispersed particles is not particularly limited, and those having a broad particle size distribution and those having a mono disperse particle size distribution may be used. Such a method is preferred for controlling the property of the coating composition that two or more kinds of dispersed particles having monodisperse particle size distributions.

Preferred examples of the polymer that can be dispersed in an aqueous solvent in the invention include a hydrophobic polymer, such as an acrylic polymer, a poly(ester) compound, a rubber compound (such as an SBR resin), a poly (urethane) compound, a poly (vinyl chloride) compound, a poly(vinyl acetate) compound, a poly (vinylidene chloride) compound and a poly(olefin) compound. The polymer may be either a linear polymer, a branched polymer or a crosslinked polymer, and may be either a so-called homopolymer formed by polymerizing a single monomer or a copolymer formed by polymerizing two or more kinds of monomers. The copolymer may be either a random copolymer or a block copolymer.

The molecular weight of the polymer is generally, in terms of number average molecular weight, from 5,000 to

1,000,000, and preferably from 10,000 to 200,000. A polymer having a too small molecular weight is insufficient in mechanical strength of the emulsion layer, and that having a too large molecular weight is not preferred due to deteriorated film forming property. Crosslinkable polymer latex is particularly preferably used.

Preferred examples of the polymer latex will be described below, but the invention is not construed as being limited thereto.

In the following description, expression is made by using the names of raw material monomers with the numbers within parentheses for percent by weight, and the molecular weight is a number average molecular weight Mn. In the case where a crosslinked structure is formed owing to the use of a polyfunctional monomer, the indication of molecular weight is omitted but is indicated as "crosslinked" because the concept of molecular weight cannot be applied to the crosslinked structure. Tg means a glass transition temperature.

P-1: Latex of MMA(70)-EA(27)-MAA(3) (Mn: 37,000, Tg: 61° C.)

P-2: Latex of MMA(70)-2EHA(20)-St(5)-AA(5) (Mn: 40,000, Tg: 59° C.)

P-3: Latex of St(50)-Bu(47)-MAA(3) (crosslinked, Tg: -17° C.)

P-4: Latex of St(68)-Bu(29)-AA(3) (crosslinked, Tg: 17° C.)

P-5: Latex of St(71)-Bu(26)-AA(3) (crosslinked, Tg: 24° C.)

P-6: Latex of St(70)-Bu(27)-IA(3) (crosslinked)

P-7: Latex of St(75)-Bu(24)-AA(1) (crosslinked, Tg: 29° C.)

P-8: Latex of St(60)-Bu(35)-DVB(3)-MAA(2) (crosslinked)

P-9: Latex of St(70)-Bu(25)-DVB(2)-AA(3) (crosslinked)

P-10: Latex of VC(50)-MAA(20)-EA(20)-AN(5)-AA(5) (Mn: 80,000)

P-11: Latex of VDC(85)-MMA(5)-EA(5)-MAA(5) (Mn: 67,000)

P-12: Latex of Et(90)-MAA(10) (Mn: 12,000)

P-13: Latex of St(70)-2EHA(27)-AA(3) (Mn: 130,000, Tg: 43° C.)

P-14: Latex of MMA(63)-EA(35)-AA(2) (Mn: 33,000, Tg: 47° C.)

P-15: Latex of St(70.5)-Bu(26.5)-AA(3) (crosslinked, Tg: 23° C.)

P-16: Latex of St(69.5)-Bu(27.5)-AA(3) (crosslinked, Tg: 20.5° C.)

In the foregoing structures, the abbreviations of monomers have the following meanings. MMA represents methyl methacrylate, EA represents ethyl acrylate, MAA represents methacrylic acid, 2EHA represents 2-ethylhexyl acrylate, St represents styrene, Bu represents butadiene, AA represents acrylic acid, DVB represents divinylbenzene, VC represents vinyl chloride, AN represents acrylonitrile, VDC represents vinylidene chloride, Et represents ethylene, and IA represents itaconic acid.

The foregoing polymer latices are commercially available, and the following polymers can be used. Examples of an acrylic polymer include Cevian A-4635, 4718 and 4601 (produced by Daicel Chemical Industries, Ltd.) and Nipol Lx 811, 814, 821, 820 and 857 (produced by Nippon Zeon Corp.), examples of a poly(ester) compound include FINETEX ES 650, 611, 675 and 850 (produced by Dainippon Ink And Chemicals, Inc.) and WD-size and WMS (produced by Eastman Chemicals, Inc.), examples of a poly (urethane) compound include HYDRAN AP 10, 20, 30 and 40 (produced by Dainippon Ink And Chemicals, Inc.), examples of a rubber compound include LACSTAR 7310K, 3307B, 4700H and 7132C (produced by Dainippon Ink And Chemicals, Inc.) and Nipol Lx 416, 410, 438C and 2507

(produced by Nippon Zeon Corp.), examples of a poly (vinyl chloride) compound include G351 and G576 (produced by Nippon Zeon Corp.), examples of a poly(vinylidene chloride) compound include L502 and L513 (produced by Asahi Kasei Corp.), and examples of a poly (olefin) compound include Chemipearl S120 and SA100 (produced by Mitsui Chemicals, Inc.).

These polymer latices may be used solely or as a mixture of two or more of them depending on necessity.

10 The polymer latex used in the invention is particularly preferably latex of a styrene-butadiene copolymer. The weight ratio of the styrene monomer unit and the butadiene monomer unit in the styrene-butadiene copolymer is preferably from 40/60 to 95/5. The proportion of the styrene monomer unit and the butadiene monomer unit in the copolymer is preferably from 60 to 90% by weight. The polymer latex of the invention preferably contains acrylic acid or methacrylic acid in an amount of from 1 to 6% by weight, more preferably from 2 to 5% by weight, based on the total amount of styrene and butadiene. The polymer latex of the invention preferably contains acrylic acid.

Preferred examples of the latex of a styrene-butadiene copolymer used in the invention include P-3 to P-8 and P-15 described in the foregoing and LACSTAR 3307B and 7132C and Nipol Lx 416, which are commercially available.

The latex of a styrene-butadiene copolymer preferably has a glass transition temperature Tg of from 10 to 30° C., and more preferably from 17 to 25° C.

In the layer containing the organic silver salt in the 30 photosensitive material of the invention, a hydrophilic polymer, such as gelatin, polyvinyl alcohol, methyl cellulose, hydroxypropyl cellulose and carboxymethyl cellulose, may be added depending on necessity. The addition amount of the hydrophilic polymer is preferably 30% by weight or less, and more preferably 20% by weight or less, based on the total binder in the layer containing the organic silver salt.

The layer containing the organic silver salt (i.e., the image forming layer) of the invention is preferably produced by 40 using polymer latex. The amount of the binder in the layer containing the organic silver salt is preferably, in terms of a weight ratio of total binder/organic silver salt, from 1/10 to 10/1, more preferably from 1/3 to 5/1, and further preferably from 1/1 to 3/1.

45 The layer containing the organic silver salt is generally a photosensitive layer (emulsion layer) containing a photosensitive silver halide, which is a photosensitive silver salt, and the weight ratio of total binder/silver halide in this case is preferably 400/1 to 5/1, and more preferably from 200/1 to 10/1.

The amount of the total binder in the image forming layer of the invention is preferably from 0.2 to 30 g/m<sup>2</sup>, more preferably from 1 to 15 g/m<sup>2</sup>, and further preferably from 2 to 10 g/m<sup>2</sup>. In the image forming layer of the invention, a crosslinking agent for crosslinking, a surface active agent for improving coating property, and the like may be added. (Preferred Solvent for Coating Composition)

A solvent for a coating composition for forming the layer containing the organic silver salt of the photosensitive material in the invention (a solvent and a dispersion medium are totally referred to as a solvent herein for simplicity) is 60 preferably an aqueous solvent containing 30% by weight or more water.

As a component other than water, an arbitrary water miscible solvent, such as methyl alcohol, ethyl alcohol, isopropyl alcohol, methylcellosolve, ethylcellosolve, dimethylformamide and ethyl acetate, may be used. The water

content of the solvent is preferably 50% by weight or more, and more preferably 70% by weight or more.

Preferred examples of the solvent composition include water, water/methyl alcohol=90/10, water/methyl alcohol=70/30, water/methyl alcohol/dimethylformamide=80/15/5, water/methyl alcohol/ethylcellosolve=85/10/5 and water/methyl alcohol/isopropyl alcohol=85/10/5 (the numerals are in terms percent by weight).

An antifoggant used in the invention will be described.

Examples of an antifoggant, a stabilizer and a stabilizer precursor that can be used in the invention include those disclosed in paragraph 0070 of JP-A-10-62899 and page 20, line 57 to page 21, line 7 of EP 0,803,764A1, compounds disclosed in JP-A-9-281637 and JP-A-9-329864, and compounds disclosed in U.S. Pat. No. 6,083,681 and European Patent No. 1,048,975.

An antifoggant that can be preferably used in the invention is an organic halogenide, and examples thereof include those disclosed in paragraphs 0111 to 0112 of JP-A-11-65012. Particularly preferred examples thereof include an organic halogenide represented by the formula (P) in JP-A-2000-284399, an organic polyhalogen compound represented by the formula (II) in JP-A-10-339934 and an organic polyhalogen compound disclosed in JP-A-2001-31644 and JP-A-2001-33911.

The organic polyhalogen compound that is preferred in the invention will be specifically described below.

The preferred polyhalogen compound in the invention includes a compound represented by the following formula (H):



wherein Q represents an alkyl group, an aryl group or a heterocyclic group, Y represents a divalent linking group, N represents 0 or 1,  $Z_1$  and  $Z_2$  each represents a halogen atom, and X represents a hydrogen atom or an electron attracting group.

In the formula (H), Q preferably represents a phenyl group substituted with an electron attracting group having a positive Hammett's substituent constant  $\sigma_p$ . With respect to the Hammett's substituent constant, *Journal of Medicinal Chemistry*, vol. 16, No. 11, p. 1207 to 1216 (1973) may be referred.

Examples of the electron attracting group include a halogen atom (such as a fluorine atom ( $\sigma_p$  value: 0.06), a chlorine atom ( $\sigma_p$  value: 0.23), a bromine atom ( $\sigma_p$  value: 0.23 and an iodine atom ( $\sigma_p$  value: 0.18)), a trihalomethyl group (such as a tribromomethyl group ( $\sigma_p$  value: 0.29), a trichloromethyl group ( $\sigma_p$  value: 0.33) and a trifluoromethyl group ( $\sigma_p$  value: 0.54)), a cyano group ( $\sigma_p$  value: 0.66), a nitro group ( $\sigma_p$  value: 0.78), an aliphatic sulfonyl group (such as a methanesulfonyl group ( $\sigma_p$  value: 0.72)), an arylsulfonyl group, a heterocyclic sulfonyl group, an aliphatic acyl group (such as an acetyl group ( $\sigma_p$  value: 0.50)), an arylacetyl group (such as a benzoyl group ( $\sigma_p$  value: 0.43)), a heterocyclic acyl group, an alkynyl group (such as a  $\text{C}\equiv\text{CH}$  group ( $\sigma_p$  value: 0.23)), an aliphatic oxycarbonyl group (such as a methoxycarbonyl group ( $\sigma_p$  value: 0.45)), an aryloxycarbonyl group (such as a phenoxy carbonyl group ( $\sigma_p$  value: 0.44)), a heterocyclic oxycarbonyl group, a carbamoyl group ( $\sigma_p$  value: 0.36), a sulfamoyl group ( $\sigma_p$  value: 0.57), a sulfoxide group, a heterocyclic group and a phosphoryl group. The  $\sigma_p$  value is preferably in a range of from 0.2 to 2.0, and more preferably in a range of from 0.4 to 1.0.

Particularly preferred examples of the electron attracting group include a carbamoyl group, an alkoxy carbonyl group,

an alkylsulfonyl group and an alkylphosphoryl group, and among these, a carbamoyl group is most preferred.

X preferably represents an electron attracting group, and more preferably represents a halogen atom, an aliphatic sulfonyl group, an arylsulfonyl group, a heterocyclic sulfonyl group, an aliphatic acyl group, an arylacetyl group, a heterocyclic acyl group, an aliphatic oxycarbonyl group, an aryloxycarbonyl group, a heterocyclic oxycarbonyl group, a carbamoyl group or a sulfamoyl group, with a halogen atom being most preferred. The halogen atom is preferably a chlorine atom, a bromine atom or an iodine atom, and more preferably a chlorine atom or a bromine atom, with a bromine atom being particularly preferred.

Y preferably represents  $-\text{C}(=\text{O})-$ ,  $-\text{SO}-$  or  $-\text{SO}_2-$ , more preferably represents  $-\text{C}(=\text{O})-$  or  $-\text{SO}_2-$ , and particularly preferably represents  $-\text{SO}_2-$ . N represents 0 or 1, and preferably represents 1.

Specific examples of the compound represented by the formula (H) in the invention will be described below.

(III-1)



(III-2)



(III-3)



(III-4)



(III-5)



(III-6)



(III-7)



(III-8)



**29**

-continued

**30**

-continued

(III-9)

5



(III-10)

10



(III-11)

15



25



(III-12)

30



(III-13)

35



(III-14)

40



(III-16)

45



(III-15)

50



(III-17)

(III-18)

(III-19)

(III-20)

(III-21)

(III-22)

(III-23)

(III-24)

60

65

65

The compound represented by the formula (H) in the invention is preferably used in an amount of from  $1 \times 10^{-4}$  to 0.5 mole, more preferably from  $1 \times 10^{-3}$  to 0.1 mole, and further preferably from  $5 \times 10^{-3}$  to 0.05 mole, per 1 mole of the nonphotosensitive silver salt in the image forming layer.

Examples of the method for adding the antifoggant into the photosensitive material include those method described for adding the reducing agent, and the organic polyhalogen compound is also preferably added in the form of a solid fine particle dispersion.

Other examples of the antifoggant include a mercury(II) salt disclosed in paragraph 0113 of JP-A-11-65021, a benzoic

## 31

acid compound disclosed in paragraph 0114 of the same publication, a formalin scavenger compound represented by the formula (S) disclosed in JP-A-2000-221634, a triazine compound disclosed in the claim 9 of JP-A-11-352624, a compound represented by the formula (III) disclosed in JP-A-6-11791, and 4-hydroxy-6-methyl-1,3,3a,7-tetraazaindene.

The photothermographic material of the invention may contain an azonium salt for preventing fogging. Examples of the azonium salt include a compound represented by the formula (XI) disclosed in JP-A-59-193447, a compound disclosed in JP-B-55-12581, and a compound represented by the formula (II) disclosed in JP-A-60-153039. The azonium salt may be any position of the photosensitive material, and it is preferably added to a layer on the surface, on which the photosensitive layer is present, and more preferably added to the layer containing the organic silver salt.

The addition of the azonium salt may be carried out in any step for preparing the coating composition, and in the case where it is added to the layer containing the organic silver salt, it may be added in any step of from preparation of the organic silver salt to preparation of the coating composition, and is preferably added in a step after preparation of the organic silver salt to a step immediately before coating. The azonium salt may be added in any method including powder, a solution or a fine particle dispersion. It may also be added in the form of a solution mixed with other additives, such as a sensitizing dye, a reducing agent and a toning agent.

The addition amount of the azonium salt in the invention maybe arbitrarily determined and is preferably from  $1 \times 10^{-6}$  to 2 mole, and more preferably from  $1 \times 10^{-3}$  to 0.5 mole, per 1 mole of silver.

In the invention, a mercapto compound, a disulfide compound and a thione compound may be added to suppress or accelerate development, to control development, to improve spectral sensitizing efficiency, and to improve storage stability before and after development. Examples thereof include compounds disclosed in paragraphs 0067 to 0069 of JP-A-10-62899, a compound represented by the formula (I) disclosed in JP-A-10-186572, specific example of which include those disclosed in paragraphs 0033 to 0052 of the same publication, and compounds disclosed in page 20, lines 36 to 56 of EP 0,803,764A1. Among these, mercapto-substituted heterocyclic aromatic compounds disclosed in JP-A-9-297367, JP-A-9-304875 and JP-A-2001-100358 are preferred.

A plasticizer and a lubricating agent that can be used in the photosensitive layer of the invention are disclosed in paragraph 0117 of JP-A-11-65021, a super high contrast agent for forming a super high contrast image and a addition method therefor that can be used therein are disclosed in paragraph 0118 of the same publication, paragraphs 0136 to 0193 of JP-A-11-223898, compounds represented by the formula (H), the formulae (1) to (3) and the formulae (A) and (B) disclosed in JP-A-2000-284399, and compounds represented by the formulae (III) to (V) disclosed in Japanese Patent Application No. 11-91652 (specific examples of which include compounds 21 to 24), and a contrast increasing accelerator that can be used therein is disclosed in paragraph 0102 of JP-A-11-65021 and paragraphs 0194 to 0195 of JP-A-11-223898.

In order to use formic acid or a formate as a forced fogging agent, it is preferably contained on the side where the image forming layer containing the photosensitive silver halide is present in an amount of 5 mmole or less, and more preferably 1 mmole or less, per 1 mole of silver.

In the case where a super high contrast agent in the photothermographic material of the invention, it is preferred

## 32

that an acid formed by hydrating diphosphorous pentaoxide or a salt thereof is used in combination.

Examples of the acid formed by hydrating diphosphorous pentaoxide or a salt thereof include metaphosphoric acid (or a salt thereof), pyrophosphoric acid (or a salt thereof), orthophosphoric acid (or a salt thereof), triphosphoric acid (or a salt thereof), tetraphosphoric acid (or a salt thereof) and a hexametaphosphoric acid (or a salt thereof).

Preferred examples of the acid formed by hydrating 10 diphosphorous pentaoxide or a salt thereof include orthophosphoric acid (or a salt thereof) and a hexametaphosphoric acid (or a salt thereof).

Specific examples of the salt include sodium orthophosphate, sodium dihydrogen orthophosphate, 15 sodium hexametaphosphate and ammonium hexametaphosphate.

The using amount of the acid formed by hydrating diphosphorous pentaoxide or a salt thereof may be arbitrarily determined according to the performance including sensitivity 20 and fogging, and is preferably from 0.1 to 500 mg/m<sup>2</sup>, and more preferably from 0.5 to 100 g/m<sup>2</sup>, in terms of a coating amount per 1 m<sup>2</sup> of the photosensitive material.

The photothermographic material of the invention may have a surface protective layer for such a purpose as 25 prevention of adhesion of the image forming layer. The surface protective layer may be a single layer or may have a multilayer structure. The surface protective layer is disclosed in paragraphs 0119 to 0120 of JP-A-11-65021 and Japanese Patent Application No. 2000-171936.

30 As a binder for the surface protective layer, gelatin can be preferably used, and it is also preferred that polyvinyl alcohol (PVA) is used or used in combination. Examples of gelatin include inert gelatin (such as Nitta Gelatin 750) and phthalated gelatin (such as Nitta Gelatin 801).

35 Examples of PVA include those disclosed in paragraphs 0009 to 0020 of JP-A-2000-171936, and preferred examples thereof include PVA-105, which is a completely saponified product, PVA-205 and PVA-335, which are partially saponified products, and MP-203, which is a modified polyvinyl alcohol, all of which are trade name of commercial products produced by Kuraray Co., Ltd.

40 The coating amount of polyvinyl alcohol in the protective layer (per one layer) in terms of an amount per 1 m<sup>2</sup> of the support is preferably from 0.3 to 4.0 g/m<sup>2</sup>, and more preferably from 0.3 to 2.0 g/m<sup>2</sup>.

45 In the case where the photothermographic material of the invention is used for printing purpose, in which dimensional change causes problems, polymer latex is preferably used in the surface protective layer and a backing layer.

50 The polymer latex is disclosed in Gosei Jusi Emulsion (Synthetic Resin Emulsion), edited by T. Okuda and H. Inagaki, published by Kobunshi Kankokai Co., Ltd. (1978), Gosei Latex no Oyo (Applications of Synthetic Latex), edited by T. Sugimura, Y. Kataoka, S. Suzuki and K.

55 Ogasawara, published by Kobunshi Kankokai Co., Ltd. (1993), and Gosei Latex no Kagaku (Chemistry of Synthetic Latex), by S. Muroi, published by Kobunshi Kankokai Co., Ltd. (1970), and specific examples thereof include latex of a copolymer of methyl methacrylate (33.5% by weight)/

60 ethyl acrylate (50% by weight)/methacrylic acid (16.5% by weight), latex of a copolymer of methyl methacrylate (47.5% by weight)/butadiene (47.5% by weight)/itaconic acid (5% by weight), latex of a copolymer of ethyl acrylate (50% by weight)/methacrylic acid (50% by weight), latex of 65 a copolymer of methyl methacrylate (58.9% by weight)/2-ethylhexyl acrylate (25.4% by weight)/styrene (8.6% by weight)/2-hydroxyethyl methacrylate (5.1% by weight)/

acrylic acid (2.0% by weight) and latex of a copolymer of methyl methacrylate (64.0% by weight)/styrene (9.0% by weight)/butyl acrylate (20.0% by weight)/2-hydroxyethyl methacrylate (5.0% by weight)/acrylic acid (2.0% by weight).

Furthermore, as a binder for the surface protective layer, a combination of polymer latex disclosed in Japanese Patent Application No. Hei 11-6872, techniques disclosed in paragraphs 0021 to 0025 of Japanese Patent Application No. Hei 11-143058, techniques disclosed in paragraphs 0027 to 0028 of Japanese Patent Application No. Hei 11-6872 and techniques disclosed in paragraphs 0023 to 0041 of Japanese Patent Application No. Hei 10-199626 may be applied.

The proportion of the polymer latex in the surface protective layer is preferably from 10 to 90% by weight, and particularly preferably from 20 to 80% by weight, based on the total amount of the binder.

The coating amount per 1 m<sup>2</sup> of the support of the total binder (including water soluble polymers and latex polymers) in the surface protective layer (per one layer) is preferably from 0.3 to 5.0 m/m<sup>2</sup>, and more preferably from 0.3 to 2.0 g/m<sup>2</sup>.

The preparation temperature of the coating composition for forming the image forming layer of the invention is preferably from 30 to 65°C., more preferably 35°C. or more and less than 60°C., and further preferably from 35 to 55°C. It is also preferred that the temperature of the coating composition for forming the image forming layer immediately after the addition of the polymer latex is maintained at a temperature of from 30 to 65°C.

The image forming layer of the invention is constituted with a single layer or two or more layers on the support. In the case where it is constituted with a single layer, it contains the organic silver salt, the photosensitive silver halide, the reducing agent and the binder, and further contains, depending on necessity, auxiliary materials, such as the toning agent, a coating assistant and other assistants. In the case where it is constituted with two or more layers, a first image forming layer (which is generally a layer adjacent to the support) contains the organic silver salt and the photosensitive silver halide, and a second image forming layer or both layers contain some other components.

In the constitution of a multi-color photothermographic photographic material, the combination of the two layers may be contained for the respective colors, and also all the components may be contained in the single layer as described in U.S. Pat. No. 4,708,928. In the case of a multi-dye multi-color photothermographic photographic material, in general, the respective emulsion layers are separately retained by using a functional or non-functional barrier layer among the respective photosensitive layers as described in U.S. Pat. No. 4,460,681.

In the photosensitive layer of the invention, various kinds of dyes and pigments (such as C.I. Pigment Blue 60, C.I. Pigment Blue 64 and C.I. Pigment Blue 15:6) may be used for improving the tone, preventing occurrence of interference fringes upon exposure with laser, and preventing irradiation. These are described in detail in WO98/36322, JP-A-10-268465 and JP-A-11-338098.

In the photothermographic material of the invention, it is preferred that an antihalation layer is provided on a side far from a light source with respect to the photosensitive layer.

The photothermographic material generally has a non-photosensitive layer in addition to the photosensitive layer. The nonphotosensitive layer can be classified into (1) a protective layer provided on the photosensitive layer (on a side far from the support), (2) an intermediate layer provided

between the plural photosensitive layer or between the photosensitive layer and the protective layer, (3) an under-coating layer provided between the photosensitive layer and the support, and (4) a backing layer provided on an opposite side to the photosensitive layer. A filter layer is provided in the photosensitive material as the layer (1) or (2). The antihalation layer is provided in the photosensitive layer as the layer (3) or (4).

The antihalation layer is described in paragraphs 0123 to 0124 of JP-A-11-65021, JP-A-11-223898, JP-A-9-230531, JP-A-10-36695, JP-A-10-104779, JP-A-11-231457, JP-A-11-352625 and JP-A-11-352626.

The antihalation layer contains an antihalation dye having absorption at the exposure wavelength. The wavelength of the exposure laser in the invention has a peak wavelength in a range of from 350 to 450 nm, and therefore, such a dye is preferably used for antihalation that absorbs light in that wavelength range.

In the case where a dye having absorption in the visible region is used for preventing halation, it is preferred that the color of the dye does substantially not remain after the image formation. It is preferred to use a means for decoloring with heat upon thermal development, and particularly it is preferred that a thermal decoloring dye and a base precursor are added to a nonphotosensitive layer to function as an antihalation layer. These techniques are described in JP-A-11-231457.

The addition amount of the decoloring dye is determined by the purpose of the dye. In general, it is preferably used in such an amount that provides an optical density (absorbance) exceeding 0.1 upon measuring at the objective wavelength. The optical density is preferably from 0.15 to 2, and more preferably from 0.2 to 1. The using amount of the dye for providing the optical density range is generally about from 0.001 to 1 g/m<sup>2</sup>.

Upon decoloring the dye, the optical density after the thermal development can be decreased to 0.1 or less. Two or more kinds of decoloring dyes may be used in combination in a thermal decoloring recording material or the photothermographic material. Similarly, two or more kinds of the base precursors may be used in combination.

In the thermal decoloration system using the decoloring dye and the base precursor, it is preferred from the standpoint of thermal decoloration to use a substance that lowers the melting point by 3°C. or more upon mixing with the base precursor described in JP-A-11-352626 (such as diphenylsulfone, 4-chlorophenyl (phenyl) sulfone) and 2-naphthyl benzoate).

In the invention, a coloring agent having an absorption maximum at from 300 to 450 nm may be added for improving silver color tone and the time-lapse change of the image. The coloring agent is described in JP-A-62-210458, JP-A-63-104046, JP-A-63-103235, JP-A-63-208846, JP-A-63-306436, JP-A-63-314535, JP-A-1-61745 and JP-A-2001-100363.

The coloring agent is generally added in an amount of from 0.1 mg/m<sup>2</sup> to 1 g/m<sup>2</sup>, and the addition layer is preferably a backing layer provided on the opposite side to the photosensitive layer.

The photothermographic material of the invention is preferably a so-called single sided photosensitive material having at least a photosensitive layer containing a silver halide emulsion on one side of a support, and having a backing layer on the other side thereof.

In the invention, a matting agent is preferably added to improve conveying property, and the matting agent is described in paragraphs 0126 to 0127 of JP-A-11-65021.

The amount of the matting agent in terms of a coating amount per 1 m<sup>2</sup> of the photosensitive material is preferably from 1 to 400 mg/m<sup>2</sup>, and more preferably from 5 to 300 mg/m<sup>2</sup>.

The shape of the matting agent in the invention may be a regular shape or an irregular shape and is preferably a regular shape with a spherical shape being more preferred. The average particle diameter thereof is preferably from 0.5 to 10  $\mu\text{m}$ , more preferably from 1.0 to 8.0  $\mu\text{m}$ , and further preferably from 2.0 to 6.0  $\mu\text{m}$ . The variation coefficient of the size distribution is preferably 50% or less, more preferably 40% or less, and further preferably 30% or less. The variation coefficient herein is a value expressed by (standard deviation of particle diameter)/(average value of particle diameter)  $\times 100$ . It is preferred to use two kinds of matting agent with small variation coefficients having average particle diameters that are different from each other by a ratio of 3 or more.

The matting degree on the emulsion surface is not limited as far as the so-called stardust phenomenon, in which small white dropouts are formed on the image part to cause leakage of light, is not caused, and it is preferably to provide a Beck's smoothness of from 30 to 2,000 seconds, and particularly preferably from 40 to 1,500 seconds. The Beck's smoothness can be conveniently obtained according to JIS P8119 (Smoothness Test Method by Beck's Testing Machine for Paper and Paperboard) and TAPPI Standard Method T479.

The matting degree of the backing layer in the invention is preferably to provide a Beck's smoothness of from 10 to 1,200 seconds, more preferably from 20 to 800 seconds, and further preferably from 40 to 500 seconds.

In the invention, the matting agent is preferably contained in the outermost layer or a layer functioning as the outermost layer of the photosensitive material or a layer in the vicinity of the outermost layer, and it is also preferably contained in a layer functioning as a so-called protective layer.

The backing layer that can be applied to the invention is described in paragraphs 0128 to 0130 of JP-A-11-65021.

The photothermographic material of the invention has a film surface pH before thermal development of 7.0 or less, and more preferably 6.6 or less. The lower limit thereof is not particularly determined and is about 3. The most preferred pH range is from 4 to 6.2.

The adjustment of the film surface pH is preferably carried out by using an organic acid, such as a phthalic acid derivative, a nonvolatile acid, such as sulfuric acid, or a volatile base, such as ammonia, from the standpoint of lowering of the film surface pH. In particular, ammonia is preferred to attain a low film surface pH since it can be removed before the coating step or the thermal development.

A nonvolatile base, such as sodium hydroxide, potassium hydroxide and lithium hydroxide, is preferably used in combination with ammonia. The method for measuring the film surface pH is described in paragraph 0123 of Japanese Patent Application No. 11-87297.

A film hardener may be used in the layers including the photosensitive layer, the protective layer and the backing layer of the invention. Examples of the film hardener include those disclosed in T. H. James, *The Theory of the Photographic Process, Fourth Edition*, p. 77 to 78, published by Macmillan Publishing Co., Inc. (1977), and preferred examples thereof include chromium alum, 2,4-dichloro-6-hydroxy-s-triazine sodium salt, N,N-ethylene-bis(vinylsulfonacetamide) and N,N-propylene-bis(vinylsulfonacetamide), and also polyvalent metallic ions disclosed on page 78 of the same literature, polyisocyanate

compounds disclosed in U.S. Pat. No. 4,281,060 and JP-A-6-208193, an epoxy compound disclosed in U.S. Pat. No. 4,791,042, and a vinylsulfone compound disclosed in JP-A-62-89048.

5 The film hardener is added in the form of a solution. The addition timing of the solution to the coating composition for forming the protective layer is generally from 180 minutes before coating to immediately before coating, and preferably 60 minutes before to 10 seconds before coating, 10 and the mixing method and the mixing conditions are not particularly limited as far as the effect of the invention is sufficiently exerted.

Specific examples of the mixing method include a method using a tank that designates a desired mean residence time 15 calculated from the addition flow rate and the supplying rate to a coater, and a method using a static mixer disclosed in N. Harnby, M. F. Edwards and A. W. Nienow (translated by K. Takahashi), *Ekitai Kongo Gijutsu* (Liquid Mixing Techniques), Chapter 8, published by Nikkan Kogyo Shimbu Co., Ltd. (1989).

20 The surface active agent that can be applied to the invention is described in paragraph 0132 of JP-A-65021, the solvent is described in paragraph 0133 of the same publication, the support is described in paragraph 0134 of the same publication, an antistatic or electroconductive layer 25 is described in paragraph 0135 of the same publication, a method for obtaining a color image is described in paragraph 0136 of the same publication, and a lubricating agent is described in paragraphs 0061 to 0064 of JP-A-11-84573 and 30 paragraphs 0049 to 0062 of Japanese Patent Application No. 11-106881.

An electroconductive layer containing a metallic oxide is 35 preferably provided in the invention. As the electroconductive material in the electroconductive layer, a metallic oxide having electroconductivity that is increased by introducing an oxygen defect or a hetero metallic defect into a metallic oxide is preferably used.

Preferred examples of the metallic oxide include ZnO, 40 TiO<sub>2</sub> and SnO<sub>2</sub>, and the addition of Al or In to ZnO, the addition of Sb, Nb, P or a halogen element to SnO<sub>2</sub>, and the addition of Nb or Ta to TiO<sub>2</sub> are preferred. In particular, SbO<sub>2</sub> having Sb added thereto is preferred.

The addition amount of the hetero atom is preferably in a range of from 0.01 to 30% by mole, and more preferably in a range of from 0.1 to 10% by mole. The shape of the metallic oxide may be either a spherical shape, an acicular shape or a tabular shape, and it is preferably acicular particles having a major axis/minor axis ratio of 2.0 or more, and more preferably from 3.0 to 50, from the standpoint of 50 endowment of electroconductivity.

The using amount of the metallic oxide is preferably in a range of from 1 to 1,000 mg/m<sup>2</sup>, more preferably in a range of from 10 to 500 mg/m<sup>2</sup>, and further preferably in a range of from 20 to 200 mg/m<sup>2</sup>. The electroconductive layer in the 55 invention may be provided on either the emulsion layer side or the backing layer side and is preferably provided between the support and the backing layer. Specific examples of the electroconductive layer in the invention are described in JP-A-7-295146 and JP-A-11-223901.

60 A fluorine surface active agent is preferably used in the invention. Specific examples of the fluorine surface active agent include compounds described in JP-A-10-197985, JP-A-2000-19680 and JP-A-2000-214554. A polymer fluorine surface active agent described in JP-A-9-281636 is also 65 preferably used. The use of a fluorine surface active agent described in Japanese Patent Application No. 2000-206560 is particularly preferred.

As a transparent support, such polyester, particularly polyethylene terephthalate, is preferably used that has been subjected to a heat treatment at a temperature range of from 130 to 185° C. to relax internal distortion remaining in the film due to biaxial stretching, so as to avoid thermal contraction caused upon thermal development. In the case of a photothermographic material for medical use, the transparent support may be colored with a blue dye (such as Dye-1 disclosed in JP-A-8-240877) or may not be colored.

Such an undercoating technique is preferably applied to the support as a water soluble polyester described in JP-A-11-84574, a styrene-butadiene copolymer described in JP-A-10-186565, and vinylidene chloride copolymers described in JP-A-2000-39684 and paragraphs 0063 to 0080 of Japanese Patent Application No. Hei 11-106881.

Those techniques can be applied to an antistatic layer and the undercoating that are described in JP-A-56-143430, JP-A-56-143431, JP-A-58-62646, JP-A-56-120519, paragraphs 0040 to 0051 of JP-A-11-84573, U.S. Pat. No. 5,575,957, and paragraphs 0078 to 0084 of JP-A-11-223898.

The photothermographic material is preferably a mono-sheet type (which can form an image on the photothermographic material without the use of an additional sheet, such as an image receiving sheet).

An antioxidant, a stabilizer, a plasticizer, an ultraviolet absorbent and a coating assistant may be added to the photothermographic material. Various kinds of the additives may be added to the photosensitive layer or the nonphotosensitive layer. They are described in WO98/36322, JP-A-10-186567 and JP-A-10-18568.

The photothermographic material of the invention may be formed by coating by any method. Specifically, various kinds of coating operation may be used, such as extrusion coating, slide coating, curtain coating, dip coating, knife coating, flow coating and extrusion coating using a hopper described in U.S. Pat. No. 2,681,294. Extrusion coating described in Stephen F. Kistler and Peter M. Schweizer, *Liquid Film Coating*, p. 399 to 536, published by Chapman & Hall, Inc. (1997), and slide coating are preferably employed, and slide coating is particularly preferably employed. Examples of the form of a slide coater used in the slide coating are disclosed in FIG. 11b.1 on page 427 of the literature. Furthermore, depending on necessity, two or more layers may be simultaneously coated according to the method described on pages 399 to 536 of the literature and the method described in U.S. Pat. No. 2,761,791 and British Patent No. 837,095.

The coating composition for the layer containing the organic silver salt in the invention is preferably a so-called thixotropic fluid. JP-A-11-52509 can be referred to for the technique.

The coating composition for the layer containing the organic silver salt preferably has a viscosity at a shearing rate of 0.1 S<sup>-1</sup> of from 400 to 100,000 mPa·s, and more preferably from 500 to 20,000 mPa·s. The viscosity at a shearing rate of 1,000 S<sup>-1</sup> is preferably from 1 to 200 mPa·s, and more preferably from 5 to 80 mPa·s.

Examples of techniques that can be applied to the photothermographic material of the invention include those described in EP803,764A1, EP883,022A1, WO98/36322, JP-A-56-62648, JP-A-58-62644, JP-A-9-43766, JP-A-9-281637, JP-A-9-297367, JP-A-9-304869, JP-A-9-311405, JP-A-9-329865, JP-A-10-10669, JP-A-10-62899, JP-A-10-69032, JP-A-10-186568, JP-A-10-90823, JP-A-10-171063, JP-A-10-186565, JP-A-10-186567, JP-A-10-186569 to 186572, JP-A-10-197974, JP-A-10-197982, JP-A-10-197983, JP-A-10-197985 to 197987, JP-A-10-207001,

JP-A-10-207004, JP-A-10-221807, JP-A-10-282601, JP-A-10-288823, JP-A-10-288824, JP-A-10-307365, JP-A-10-312038, JP-A-10-339934, JP-A-11-7100, JP-A-11-15105, JP-A-11-24200, JP-A-11-24201, JP-A-11-30832, JP-A-11-84574, JP-A-11-65021, JP-A-11-109547, JP-A-11-125880, JP-A-11-129629, JP-A-11-133536 to 133539, JP-A-11-133542, JP-A-11-133543, JP-A-11-223898, JP-A-11-352627, JP-A-11-305377, JP-A-11-305378, JP-A-11-305384, JP-A-11-305380, JP-A-11-316435, JP-A-11-327076, JP-A-11-338098, JP-A-11-338099, JP-A-11-343420 and Japanese Patent Application Nos. 2000-187298, 2000-10229, 200-47345, 2000-206642, 2000-98530, 2000-98531, 2000-112059, 2000-112060, 2000-112104, 2000-112064 and 2000-171936.

15 The photosensitive material of the invention is preferably packed with such a packing material that is low in oxygen permeability and/or moisture permeability in order to suppress change in photographic performance during storage before use.

20 The oxygen permeability at 25° C. is preferably 50 mL/atm·m<sup>2</sup>·day or less, more preferably 10 mL/atm·m<sup>2</sup>·day or less, and further preferably 1.0 mL/atm·m<sup>2</sup>·day or less. The moisture permeability is preferably 10 g/atm·m<sup>2</sup>·day or less, more preferably 5 g/atm·m<sup>2</sup>·day or less, and further preferably 1 g/atm·m<sup>2</sup>·day or less.

25 Specific examples of the packing material that is low in oxygen permeability and/or moisture permeability include packing materials described in JP-A-8-254793 and JP-A-2000-206653.

30 The photothermographic material of the invention may be developed by any method, and in general, a photothermographic material having been imagewise exposed is heated to accomplish development. The developing temperature is preferably from 80 to 250° C., more preferably from 100 to 140° C., and further preferably from 110 to 130° C. The developing time is preferably from 1 to 60 seconds, more preferably from 3 to 30 seconds, further preferably from 5 to 25 seconds, and particularly preferably from 7 to 15 seconds.

35 40 45 50 As the method of thermal development, any of a drum heater or a plate heater may be used, and the use of a plate heater is preferred. As a thermal developing method using a plate heater, a method described in JP-A-11-133572 is preferred, which uses such a developing apparatus that provides a visible image by contacting a photothermographic material having a latent image formed therein with a heating means in a thermal developing part, in which the heating means contains a plate heater, plural pressure rollers are arranged along one surface of the plate heater as opposed thereto, and thermal development is attained by passing the photothermographic material between the pressure rollers and the plate heater. It is preferred that the plate heater is divided into two to six stages, and the temperature of the tip end part is lowered by about from 1 to 10° C.

55 60 65 For example, four sets of plate heaters that can be independently controlled in temperature are provided, and the temperatures thereof are controlled to 112° C., 119° C., 121° C. and 120° C., respectively. Such a method is also described in JP-A-54-30032, by which water content and an organic solvent contained in the photothermographic material can be removed out of the system, and the support can be prevented from change in shape due to rapid heating of the photothermographic material.

65 The photosensitive material of the invention exerts the characteristics thereof upon exposure for a short period of time with light of a high illuminance of 1 mW/mm<sup>2</sup> or more.

Upon exposure at such a high illuminance, sufficient sensitivity can be obtained by the photothermographic material of the invention containing the silver halide having a high silver iodide content and the nonphotosensitive organic silver salt. In other words, the photosensitive material of the invention can attain high sensitivity with high illuminance exposure in comparison to low illuminance exposure.

The illuminance is more preferably from 2 to 50 mW/mm<sup>2</sup>, and further preferably from 10 to 50 mW/mm<sup>2</sup>.

While any light source may be used as far as the conditions are satisfied, it is preferably attained by using laser light.

Examples of the laser light that can be preferably used in the invention include that emitted from a gas laser (such as Ar<sup>+</sup> and Kr), a YAG laser, a dye laser and a semiconductor laser. Furthermore, a laser and a secondary harmonic wave generating element can also be used. More preferred examples include a semiconductor laser emitting blue to ultraviolet light, and further preferred examples include a semiconductor laser having a light emission peak at a wavelength range of from 350 to 450 nm, further preferably in a wavelength range of from 390 to 430 nm. Examples of the high output semiconductor laser emitting blue to ultraviolet light include a semiconductor laser NLHV 3000E produced by Nichia Corp., and for example a laser having an output of 35 mW at a wavelength of 405 nm has been released. A high illuminance at a wavelength of from 390 to 430 nm, which is a particularly preferred wavelength for the photosensitive material of the invention, can be obtained by using the laser light.

Examples of a laser imager for medical use having an exposing part and a thermal developing part include Dry Imager FM-DP L by Fuji Medical Systems Inc.

FM-DP L is described in *Fuji Medical Review*, No. 8, p. 39 to 55, and the technique therein can be applied to a laser imager for the photothermographic material of the invention. The photothermographic material of the invention can also be applied to that for a laser imager used in the AD Network, which has been proposed by Fuji Medical Systems Inc. as a network system that complies with the DICOM Standard.

The photothermographic material of the invention forms a monochrome image with a silver image, and is preferably used as a photothermographic material for medical diagnosis, a photothermographic material for industrial photography, a photothermographic material for printing, and a photothermographic material for COM.

## EXAMPLES

The invention will be specifically described with reference to the following examples, but the invention is not construed as being limited thereto.

### Example 1

#### (Production of Photothermographic Material 1) (Preparation Example of PET Support)

PET having an intrinsic viscosity IV of 0.66 (measured in phenol/tetrachloroethane (6/4 by volume) at 25° C.) was obtained by the ordinary method using terephthalic acid and ethylene glycol. After forming the same into pellets, it was dried at 130° C. for 4 hours and was melted at 300° C., to which the following Dye BB having the following structure was added in an amount of 0.04% by weight. It was extruded from a T die and then rapidly cooled to produce an unstretched film having such a thickness that provided a thickness after heat fixing of 175 μm.

Dye BB:



The film was stretched in the machine direction by 3.3 times using rolls having different peripheral velocities and then stretched in the transversal direction by 4.5 times using a tenter. The temperatures upon stretching were 110° C. and 130° C., respectively. Thereafter, the film was heat-fixed at 240° C. for 20 seconds, and then relaxed in the transversal direction by 4% at the same temperature. The part clucked by the tenter was slit out, and then the both ends were knurled, followed by wound at 4 kg/cm<sup>2</sup>, to obtain a roll of a film having a thickness of 175 μm.

(Surface Corona Treatment)

The both surfaces of the support were treated at room temperature and 20 m/min by using a solid state corona treatment machine, 6 KVA Model produced by Piller Inc. It was found from the read values of electric current and voltage that a treatment of 0.375 kV·A·min/m<sup>2</sup> was applied to the support. Upon the treatment, the treating frequency was 9.6 kHz, and the gap clearance between the electrode and the dielectric roll was 1.6 mm.

(Preparation Example of Undercoated Support)

(Preparation of Coating Composition for Under Coating)

|                                                                                                                                                                                                                                  |        |
|----------------------------------------------------------------------------------------------------------------------------------------------------------------------------------------------------------------------------------|--------|
| 40                                                                                                                                                                                                                               |        |
| <u>Composition (1)</u><br>(for undercoating on the photosensitive layer side)                                                                                                                                                    |        |
| Pesresin A-520 (30% by weight solution)<br>produced by Takamatsu Oil & Fat Co., Ltd.                                                                                                                                             | 59 g   |
| Polyethylene glycol monononylphenyl ether<br>(average oxide number: 8.5) 10% by weight solution<br>MP-1000 (polymer fine particles)<br>(average particle diameter: 0.4 μm)<br>produced by Soken Chemical & Engineering Co., Ltd. | 5.4 g  |
| Distilled water                                                                                                                                                                                                                  | 0.91 g |
| Composition (2)<br>(for first layer on the backing layer side)                                                                                                                                                                   | 935 mL |
| Styrene-butadiene copolymer latex<br>(solid content: 40% by weight, styrene/butadiene weight ratio: 68/32)                                                                                                                       | 158 g  |
| 55 2,4-dichloro-6-hydroxy-S-triazine sodium salt<br>(8% by weight aqueous solution)                                                                                                                                              | 20 g   |
| Sodium laurylbenzenesulfonate<br>(1% by weight aqueous solution)                                                                                                                                                                 | 10 mL  |
| Distilled water                                                                                                                                                                                                                  | 854 mL |
| Composition (3)<br>(for second layer on the backing surface side)                                                                                                                                                                |        |
| SnO <sub>2</sub> /SbO<br>(weight ratio: 9/1, average particle diameter: 0.038 μm,<br>17% by weight dispersion)                                                                                                                   | 84 g   |
| 55 Gelatin (10% by weight aqueous solution)                                                                                                                                                                                      | 89.2 g |
| Metolose TC-5 (2% by weight aqueous solution)<br>produced by Shin-Etsu Chemical Co., Ltd.                                                                                                                                        | 8.6 g  |
| MP-1000                                                                                                                                                                                                                          | 0.01 g |

-continued

produced by Soken Chemical & Engineering Co., Ltd.  
Sodium dodecylbenzenesulfonate

|                                                 |        |
|-------------------------------------------------|--------|
| (1% by weight aqueous solution)                 | 10 mL  |
| NaOH (1% by weight)                             | 6 mL   |
| Proxel produced by Imperial Chemical Industries | 1 mL   |
| Distilled water                                 | 805 mL |

## (Production of Undercoated Support)

Both the surfaces of the biaxially stretched polyethylene terephthalate support having a thickness of 175  $\mu\text{m}$  were subjected to the foregoing corona treatment. The coating composition (1) for undercoating was coated on one surface thereof (photosensitive layer side) with a wire bar to a wet coated amount of 6.6 mL/m<sup>2</sup> (per one surface) and then dried at 180° C. for 5 minutes, and then the coating composition (2) for undercoating was coated on the opposite surface (backing layer side) to a wet coated amount of 5.7 mL/m<sup>2</sup> and then dried at 180° C. for 5 minutes. The coating composition (3) was further coated on the back surface (backing layer side) to a wet coated amount of 7.7 mL/m<sup>2</sup> and then dried at 180° C. for 6 minutes to produce an undercoated support.

## (Preparation of Backing Layer Coating Composition)

## (Preparation of Coating Composition for Antihalation Layer)

17 g of gelatin, 9.6 g of polyacrylamide, 1.5 g of monodisperse polymethyl methacrylate fine particles (average particle diameter: 8  $\mu\text{m}$ , particle size standard deviation: 0.4), 0.03 g of benzoisothiazoline, 2.2 g of sodium polyethylenesulfonate, 0.1 g of a blue dye compound 1 (having a structure described later), 0.1 g of a yellow dye compound 1 (having a structure described later), and 844 mL of water were mixed to prepare a coating composition for an antihalation layer.

## (Preparation of Coating Composition for Protective Layer on Back Surface)

In a container maintained at 40° C., 50 g of gelatin, 0.2 g of sodium polystyrenesulfonate, 2.4 g of N,N-ethylene-bis(vinylsulfonacetamide), 1 g of sodium t-octylphenoxyethoxyethanesulfonate, 30 mg of benzoisothiazoline, 37 mg of a fluorine surface active agent (F-1: N-perfluoroctylsulfonyl-N-propylalanine potassium salt), 150 mg of a fluorine surface active agent (F-2: polyethylene glycol mono(N-perfluoroctylsulfonyl-N-propyl-2-aminoethyl) ether (average polymerization degree of ethyleneoxide: 15)), 64 mg of a fluorine surface active agent (F-3: having a structure described later), 32 mg of a fluorine surface active agent (F-4: having a structure described later), 10 mg of a fluorine surface active agent (F-7: having a structure described later), 5 mg of a fluorine surface active agent (F-8: having a structure described later) 8.8 g of an acrylic acid/ethyl acrylate copolymer (copolymerization ratio: 5/95 by weight), 0.6 g of Aerosol OT (produced by American Cyanamid Co., Ltd.), 1.8 g in terms of liquid paraffin of an emulsion of liquid paraffin, and 950 mg of water were mixed to obtain a coating composition for the protective layer on the back surface.

## (Preparation of Silver Halide Emulsion)

## (Preparation of Silver Halide Emulsion 1)

3.1 mL of 1% by weight potassium bromide solution was added to 1,420 mL of distilled water, and 3.5 mL of sulfuric acid having a concentration of 0.5 mol/L and 36.5 g of phthalated gelatin were added thereto to obtain a solution. The solution was maintained at a liquid temperature at 30° C. under stirring in a stainless steel reaction vessel, and the

total amounts of a solution A, which was obtained by diluting 22.22 g of silver nitrate with distilled water to make 95.4 mL, and a solution B, which was obtained by diluting 15.3 g of potassium bromide and 0.8 g of potassium iodide with distilled water to make 97.4 mL, were added thereto over 45 seconds at constant flow rates. Thereafter, 10 mL of a 3.5% by weight hydrogen peroxide aqueous solution was added, and 10.8 mL of a 10% by weight benzoimidazole aqueous solution was further added.

Furthermore, a solution C, which was obtained by diluting 51.86 g of silver nitrate with distilled water to make 317.5 mL, and a solution D, which was obtained by diluting 44.2 g of potassium bromide and 2.2 g of potassium iodide with distilled water to make 400 mL, were prepared. The total amount of the solution C was added over 20 minutes at a constant flow rate, and the solution D was added by the controlled double jet (CDJ) method under maintaining the pAg at 8.1. The total amount of  $1\times 10^{-4}$  mole of iridium (III) hexachloride per 1 mole of silver was added after 10 minutes from the start of the addition of the solutions C and D. After 5 seconds from the completion of the addition of the solution C, the total amount of  $3\times 10^{-4}$  mole of an aqueous solution of potassium iron (II) hexacyanide per 1 mole of silver was added. The pH was adjusted to 3.8 by using sulfuric acid having a concentration of 0.5 mole/L, and stirring was terminated, followed by subjecting to sedimentation, desalination and water washing steps.

The pH was adjusted to 5.9 by using a sodium hydroxide solution having a concentration of 1 mole/L to prepare a silver halide dispersion having pAg 8.0.

The silver halide dispersion was maintained at 38° C. under stirring, and 5 mL of a 0.34% by weight methanol solution of 1,2-benzoisothiazolin-3-one was added, followed by increasing the temperature to 47° C. 20 minutes after the temperature increase, sodium benzenethiosulfonate in the form of a methanol solution was added in an amount of  $7.6\times 10^{-5}$  mole per 1 mole of silver, and further 5 minutes after, a tellurium sensitizer C (having a structure described later) in the form of a methanol solution was added in an amount of  $2.9\times 10^{-4}$  mole per 1 mole of silver, followed by aging for 91 minutes.

1.3 mL of a 0.8% by weight methanol solution of N,N'-dihydroxy-N"-diethylmelamine was added, and further 4 minutes after,  $4.8\times 10^{-3}$  mole per 1 mole of silver of 5-methyl-2-mercaptopbenzimidazole in the form of a methanol solution,  $5.4\times 10^{-3}$  mole per 1 mole of silver of 1-phenyl-2-heptyl-5-mercaptop-1,3,4-triazole in the form of a methanol solution, and  $8.5\times 10^{-3}$  mole per 1 mole of silver of 1-(3-methylureido)-5-mercaptotetrazole sodium salt in the form of an aqueous solution were added to produce a silver halide emulsion 1.

The particles in the thus prepared silver halide emulsion were silver iodobromide particles having an average sphere-equivalent diameter of 0.040  $\mu\text{m}$  and a variation coefficient of the sphere-equivalent diameter of 18%. The particle size and other parameters were obtained from an average of measurements of 1,000 particles with an electron microscope.

## (Preparation of Mixed Emulsion A for Coating)

The silver halide emulsion 1 was dissolved, and a 1% by weight aqueous solution of benzothiazolium iodide was added in an amount of  $7\times 10^{-3}$  mole per 1 mole of silver. Water was added in such an amount that the content of the silver halide in terms of silver became 38.2 g per 1 kg of the mixed emulsion for coating, and 1-(3-methylureido)-5-mercaptotetrazole sodium salt was added in such an amount that the amount thereof became 0.34 g per 1 kg of the mixed emulsion for coating.

## (Preparation of Fatty Acid Silver Salt Dispersion)

87.6 kg of behenic acid (Edenor C22-85R, a trade name, produced by Henkel Co., Ltd.), 423 L of distilled water, 49.2 L of an NaOH aqueous solution having a concentration of 5 mole/L, and 120 L of t-butyl alcohol were mixed and reacted at 75° C. for 1 hour to obtain a sodium behenate solution. Separately, 206.2 L of an aqueous solution of 40.4 kg of silver nitrate (pH 4.0) was prepared and maintained at 10° C. A reaction vessel containing 635 L of distilled water and 30 L of t-butyl alcohol was maintained at 30° C., and the total amount of the sodium behenate solution and the total amount of the silver nitrate aqueous solution were added under stirring at constant flow rates over 93 minutes and 15 seconds, and 90 minutes, respectively.

At this time, only the silver nitrate aqueous solution was added in the initial 11 minutes period of the addition of the silver nitrate aqueous solution, and then the sodium behenate solution was started to be added. In the period of 14 minutes and 15 seconds after the completion of the addition of the silver nitrate aqueous solution, only the sodium behenate solution was added. At this time, the temperature inside the reaction vessel was 30° C., and the external temperature was controlled to maintain the liquid temperature constant.

The temperature of the piping of the addition system of the sodium behenate solution was maintained by circulating warm water in the outside layer of the dual pipe, whereby the liquid temperature at the outlet of the tip end of the addition nozzle was adjusted to 75° C. The temperature of the piping of the addition system of the silver nitrate aqueous solution was maintained by circulating cold water in the outside layer of the dual pipe. The addition position of the sodium behenate solution and the addition position of the silver nitrate aqueous solution were arranged at the symmetric positions with respect to the stirring axis and were adjusted in height to prevent from contacting with the reaction liquid.

After completing the addition of the sodium behenate solution, the reaction solution was allowed to stand at that temperature for 20 minutes under stirring, and the temperature thereof was then increased to 35° C. over 30 minutes, followed by aging for 210 minutes. Immediately after completing the aging, a solid content was filtered off by centrifugal filtration, and the solid content was washed with water until the electroconductivity of the filtrate became 30  $\mu\text{S}/\text{cm}$ . Thus, silver behenate was obtained. The resulting solid content was not dried and stored in the form of a wet cake.

The shape of the resulting silver behenate particles were evaluated by electron microscope observation, and thus they were squamous crystals having  $a=0.14 \mu\text{m}$ ,  $b=0.4 \mu\text{m}$  and  $c=0.6 \mu\text{m}$  in terms of average values, an average aspect ratio of 5.2, an average sphere-equivalent diameter of  $0.52 \mu\text{m}$ , and a variation coefficient of the sphere-equivalent diameter of 15%. (a, b and c were determined by the foregoing definition.)

19.3 kg of polyvinyl alcohol (PVA-217, a trade name) and water were added to a wet cake in an amount corresponding to 260 kg of a dry solid content to make a total amount 1,000 kg, and the mixture was formed into a slurry with dissolver blades, followed by subjecting to preliminary dispersion with a pipeline mixer (Model PM-10, produced by Mizuho Industrial Co., Ltd.).

The stock solution after subjecting to the preliminary dispersion was treated three times with a dispersing machine (Microfluidizer M-610, a trade name, produced by Microfluidex International Corp., using Z type interaction chamber) adjusted to have a pressure of 1,260 kg/cm<sup>2</sup> to

obtain a silver behenate dispersion. The cooling operation was set at a dispersion temperature of 18° C. by installing corrugated tube heat exchangers before and after the interaction chamber to adjust the temperature of the cooling medium.

## (Preparation of Reducing Agent Dispersion)

## (Preparation of Reducing Agent 2 Dispersion)

10 kg of water was added to 10 kg of the reducing agent (6,6'-di-t-butyl-4,4'-dimethyl-2,2'-butyldenediphenol) and 16 kg of a 10% by weight aqueous solution of modified polyvinyl alcohol (Poval MP203, produced by Kuraray Co., Ltd.), followed by well mixing, to prepare a slurry.

The slurry was transported with a diaphragm pump and dispersed for 3 hours and 30 minutes in a transverse sand mill (UVM-2, produced by Imex Co., Ltd.) filled with zirconia beads having an average diameter of 0.5 mm. Thereafter, 0.2 g of benzoisothiazolinone sodium salt and water were added to adjust the concentration of the reducing agent to 25% by weight to obtain a reducing agent 2 dispersion.

The reducing agent particles contained in the reducing agent dispersion had a median diameter of  $0.40 \mu\text{m}$  and a maximum particle diameter of  $1.5 \mu\text{m}$  or less. The resulting reducing agent dispersion was filtered with a polypropylene filter having a pore size of  $3.0 \mu\text{m}$  to remove foreign matters, such as dusts, and then stored.

## (Preparation of Hydrogen Bonding Compound 1 Dispersion)

10 kg of water was added to 10 kg of the hydrogen bonding compound 1 (tri (4-t-butylphenyl)phosphineoxide) and 16 kg of a 10% by weight aqueous solution of modified polyvinyl alcohol (Poval MP203, produced by Kuraray Co., Ltd.), followed by well mixing, to prepare a slurry.

The slurry was transported with a diaphragm pump and dispersed for 3 hours and 30 minutes in a transverse sand mill (UVM-2, produced by Imex Co., Ltd.) filled with zirconia beads having an average diameter of 0.5 mm. Thereafter, 0.2 g of benzoisothiazolinone sodium salt and water were added to adjust the concentration of the hydrogen bonding compound to 25% by weight to obtain a hydrogen bonding compound 1 dispersion.

The hydrogen bonding compound particles contained in the hydrogen bonding compound dispersion had a median diameter of  $0.35 \mu\text{m}$  and a maximum particle diameter of  $1.5 \mu\text{m}$  or less. The resulting hydrogen bonding compound dispersion was filtered with a polypropylene filter having a pore size of  $3.0 \mu\text{m}$  to remove foreign matters, such as dusts, and then stored.

## (Preparation of Development Accelerating Agent 1 Dispersion)

10 kg of water was added to 10 kg of the development accelerating agent (having a structure described later) and 20 kg of a 10% by weight aqueous solution of modified polyvinyl alcohol (Poval MP203, produced by Kuraray Co., Ltd.), followed by well mixing, to prepare a slurry.

The slurry was transported with a diaphragm pump and dispersed for 3 hours and 30 minutes in a transverse sand mill (UVM-2, produced by Imex Co., Ltd.) filled with zirconia beads having an average diameter of 0.5 mm. Thereafter, 0.2 g of benzoisothiazolinone sodium salt and water were added to adjust the concentration of the development accelerating agent to 20% by weight to obtain a development accelerating agent 1 dispersion.

The development accelerating agent particles contained in the development accelerating agent dispersion had a median diameter of  $0.48 \mu\text{m}$  and a maximum particle diameter of  $1.4 \mu\text{m}$  or less. The resulting development accelerating agent

45

dispersion was filtered with a polypropylene filter having a pore size of  $3.0\text{ }\mu\text{m}$  to remove foreign matters, such as dusts, and then stored.

Solid dispersions of the development accelerating agent 2, the development accelerating agent 3 and the toning agent 1 (each having structures described later) were prepared by dispersing in the same manner as in the development accelerating agent 1 to prepare 20% by weight dispersions.

(Preparation of Polyhalogen Compound)

(Preparation of Organic Polyhalogen Compound 1 Dispersion)

10 kg of the organic polyhalogen compound 1 (tribromomethanesulfonylbenzene), 10 kg of a 20% by weight aqueous solution of modified polyvinyl alcohol (Poval MP203, produced by Kuraray Co., Ltd.), 0.4 kg of a 20% by weight aqueous solution of sodium triisopropyl-naphthalenesulfonate and 14 kg of water were well mixed to prepare a slurry.

The slurry was transported with a diaphragm pump and dispersed for 5 hours in a transverse sand mill (UVM-2, produced by Imex Co., Ltd.) filled with zirconia beads having an average diameter of 0.5 mm. Thereafter, 0.2 g of benzoisothazolinone sodium salt and water were added to adjust the concentration of the organic polyhalogen compound to 26% by weight to obtain a organic polyhalogen compound 1 dispersion.

The organic polyhalogen compound particles contained in the organic polyhalogen compound dispersion had a median diameter of  $0.41\text{ }\mu\text{m}$  and a maximum particle diameter of  $2.0\text{ }\mu\text{m}$  or less. The resulting organic polyhalogen compound dispersion was filtered with a polypropylene filter having a pore size of  $10.0\text{ }\mu\text{m}$  to remove foreign matters, such as dusts, and then stored.

(Preparation of Organic Polyhalogen Compound 2 Dispersion)

10 kg of the organic polyhalogen compound 2 (N-butyl-3-tribromomethanesulfonylbenzamide), 20 kg of a 10% by weight aqueous solution of modified polyvinyl alcohol (Poval MP203, produced by Kuraray Co., Ltd.) and 0.4 kg of a 20% by weight aqueous solution of sodium triisopropyl-naphthalenesulfonate were well mixed to prepare a slurry.

The slurry was transported with a diaphragm pump and dispersed for 5 hours in a transverse sand mill (UVM-2, produced by Imex Co., Ltd.) filled with zirconia beads having an average diameter of 0.5 mm. Thereafter, 0.2 g of benzoisothazolinone sodium salt and water were added to adjust the concentration of the organic polyhalogen compound to 30% by weight to obtain a organic polyhalogen compound 2 dispersion.

The organic polyhalogen compound particles contained in the organic polyhalogen compound dispersion had a median diameter of  $0.40\text{ }\mu\text{m}$  and a maximum particle diameter of  $1.3\text{ }\mu\text{m}$  or less. The resulting organic polyhalogen compound dispersion was filtered with a polypropylene filter having a pore size of  $3.0\text{ }\mu\text{m}$  to remove foreign matters, such as dusts, and then stored.

(Preparation of Phthalazine Compound 1 Solution)

8 kg of modified polyvinyl alcohol MP203, produced by Kuraray Co., Ltd., was dissolved in 174.57 kg of water, and 3.15 kg of a 20% by weight aqueous solution of sodium triisopropylnaphthalenesulfonate and 14.28 kg of a 70% by weight aqueous solution of the phthalazine compound 1 (6-isopropylphthalazine) were added to obtain a 5% by weight solution of the phthalazine compound 1.

46

(Preparation of Mercapto Compound)

(Preparation of Mercapto Compound 2 Aqueous Solution)

20 g of a mercapto compound 2 (1-(3-methylureido)-5-mercaptopotetrazole sodium salt) was dissolved in 980 g of water to obtain a 2.0% by weight aqueous solution.

(Preparation of Pigment 1 Dispersion)

250 g of water was added to 64 g of C.I. Pigment Blue 60 and 6.4 g of Demol N, produced by Kao Corp., followed by well mixing, to prepare a slurry. 800 g of zirconia beads having an average particle diameter of 0.5 mm were prepared and placed in a vessel along with the slurry, and they were dispersed for 25 hours in a dispersing apparatus (1/4G sand grinder mill, produced by Imex Co., Ltd.). The concentration of the pigment was adjusted to 5% by weight by adding water to obtain a pigment 1 dispersion. The average particle diameter of the pigment particles contained in the pigment dispersion was  $0.21\text{ }\mu\text{m}$ .

(Preparation of SBR Latex Liquid)

The SBR latex was prepared in the following manner.

287 g of distilled water, 7.73 g of a surface active agent (Pionin A-43-S, produced by Takemoto Oil and Fat Co., Ltd., solid content: 48.5%), 14.06 mL of 1 mol/L NaOH solution, 0.15 g of tetrasodium ethylenediamine tetraacetate, 255 g of styrene, 11.25 g of acrylic acid and 3.0 g of tert-dodecylmercaptane were placed in a polymerization vessel of a gas monomer reaction apparatus (Model TAS-2J, produced by Taiatsu Techno Corp.), and the reaction vessel was sealed and stirred at a stirring rate of 200 rpm. The vessel was evacuated with a vacuum pump and replaced

several times with nitrogen gas, and then 108.75 g of 1,3-butadiene was pressed thereinto, followed by increasing the interior temperature to  $60^\circ\text{ C}$ . A liquid obtained by dissolving 1.875 g of ammonium persulfate in 50 mL of water was added thereto, followed by stirring for 5 hours. The temperature was then increased to  $90^\circ\text{ C}$ ., followed by stirring for 3 hours, and after completing the reaction, the temperature was lowered to room temperature. 1 mole/L NaOH and 1 mole/L NH4OH were added to make a ratio of  $\text{Na}^+$  ion/ $\text{NH}_4^+$  ion of 1/5.3 (by mole) to adjust the pH to 8.4.

Thereafter, the mixture was filtered with a polypropylene filter having a pore size of  $1.0\text{ }\mu\text{m}$  to remove foreign matters, such as dusts, and then stored, so as to obtain 774.7 g of SBR latex. The measurement of a halogen ion with ion chromatography revealed that the chloride ion concentration was 3 ppm. The concentration of the chelating agent measured by high performance liquid chromatography was 145 ppm.

The latex had an average particle diameter of 90 nm, a glass transition temperature  $T_g$  of  $17^\circ\text{ C}$ ., a solid content of 44% by weight, an equilibrium water content at  $25^\circ\text{ C}$ . and 50 60% RH of 0.6% by weight, an ionic conductivity of 4.80 mS/cm (the measurement of the ionic conductivity was carried out by using a conductivity meter CM-30S, produced by Toa Electronics Ltd. for the latex stock liquid (44% by weight) at  $25^\circ\text{ C}$ .), and pH 8.4.

55 SBR latex having a different  $T_g$  was prepared in the similar manner with appropriate variation of the ratio of styrene and butadiene.

(Preparation of Coating Composition for Emulsion Layer (Photosensitive Layer) 1)

60 The components obtained in the foregoing, 1,000 g of the fatty acid silver salt dispersion, 276 mL of water, 3.2 g of the organic polyhalogen compound 1 dispersion, 8.7 g of the organic polyhalogen 2 dispersion, 173 g of the phthalazine compound 1 dispersion, 1,082 g of the SBR latex ( $T_g$ :  $17^\circ\text{ C}$ .), 155 g of the reducing agent 2 dispersion, 55 g of the hydrogen bonding compound 1 dispersion, 1 g of the development accelerating agent 1 dispersion, 2 g of the develop-

ment accelerating agent 2 dispersion, 3 g of the development accelerating agent 3 dispersion, 2 g of the toning agent 1 dispersion, and 6 mL of the mercapto compound 2 aqueous solution were added in this order, and 117 g of the silver halide mixed emulsion was added immediately before coating, followed by well mixing, to obtain a coating composition for an emulsion layer, which was directly transported to a coating die for coating.

The coating composition for an emulsion layer had a viscosity measured with a B-type viscometer of Tokyo Keiki of 40 mPa·s at 40° C. (No. 1 rotor at 60 rpm).

The viscosity of the coating composition measured with RFS Fluid Spectrometer produced by Rheometrics Far East Co., Ltd. was 530, 144, 96, 51 and 28 mPa·s at a shearing rate of 0.1, 1, 10, 100 and 1,000 1/sec, respectively.

The zirconium amount in the coating composition was 0.25 mg per 1 g of silver.

(Preparation of Coating Composition for Intermediate Layer on Emulsion Layer Side)

To 1,000 g of polyvinyl alcohol PVA-205 (produced by Kuraray Co., Ltd.), 272 g of a 5% by weight dispersion of a pigment, 4,200 mL of a 19% by weight liquid of latex of a methyl methacrylate/styrene/butyl acrylate/hydroxyethyl acrylate/acrylic acid copolymer (copolymerization ratio: 64/9/20/5/2), 27 mL of a 5% by weight aqueous solution of Aerозол OT (produced by American Cyanamid Co., Ltd.) and 135 mL of a 20% by weight aqueous solution of diammomium phthalate, water was added to make a total amount of 10,000 g, and the pH was adjusted to 7.5 with NaOH, so as to obtain a coating composition for an intermediate layer, which was transported to a coating die to make 9.1 mL/m<sup>2</sup>.

The coating composition had a viscosity measured with a B-type viscometer of Tokyo Keiki of 58 mPa·s at 40° C. (No. 1 rotor at 60 rpm).

(Preparation of Coating Composition for First Layer of Protective Layer on Emulsion Layer Side)

64 g of inert gelatin was dissolved in water, and 80 g of a 27.5% by weight liquid of latex of a methyl methacrylate/styrene/butyl acrylate/hydroxyethyl acrylate/acrylic acid copolymer (copolymerization ratio: 64/9/20/5/2), 23 mL of a 10% by weight methanol solution of phthalic acid, 23 mL of a 10% by weight aqueous solution of 4-methylphthalic acid, 28 mL of sulfuric acid having a concentration of 0.5 mole/L, 5 mL of a 5% by weight aqueous solution of Aerозол OT (produced by American Cyanamid Co., Ltd.), 0.5 g of phenoxyethanol and 0.1 g of benzoisothiazoline were added thereto. Water was added to make a total amount of 750 g to prepare a coating composition. 26 mL of a 4% by weight solution of chromium alum was mixed by a static mixer immediately before coating, and the mixture was transported to a coating die to make 18.6 mL/m<sup>2</sup>.

The coating composition had a viscosity measured with a B-type viscometer of Tokyo Keiki of 20 mPa·s at 40° C. (No. 1 rotor at 60 rpm).

(Preparation of Coating Composition for Second Layer of Protective Layer on Emulsion Layer Side)

80 g of inert gelatin was dissolved in water, and 102 g of a 27.5% by weight liquid of latex of a methyl methacrylate/styrene/butyl acrylate/hydroxyethyl acrylate/acrylic acid copolymer (copolymerization ratio: 64/9/20/5/2), 3.2 mL of a 5% by weight solution of a fluorine surface active agent (F-1: N-perfluoroctylsulfonyl-N-propylalanine potassium salt), 32 mL of a 2% by weight aqueous solution of a fluorine surface active agent (F-2: polyethylene glycol mono (N-perfluoroctylsulfonyl-N-propyl-2-amonoethyl) ether (average polymerization degree of ethyleneoxide: 15)), 3

5 mL of a 5% by weight solution of a fluorine surface active agent (F-5 having a structure described later), 10 mL of a 2% by weight solution of a fluorine surface active agent (F-6 having a structure described later), 23 mL of a 5% by weight aqueous solution of Aerозол OT (produced by American Cyanamid Co., Ltd.), 4 g of polymethyl methacrylate fine particles (average particle diameter: 0.7 μm), 21 g of polymethyl methacrylate fine particles (average particle diameter: 4.5 μm), 1.6 g of 4-methylphthalic acid, 4.8 g of phthalic acid, 44 mL of sulfuric acid having a concentration of 0.5 mole/L and 10 mg of benzoisothiazoline were added thereto. Water was added to make a total amount of 650 g, and 445 mL of an aqueous solution containing 4% by weight of chromium alum and 0.67% by weight of phthalic acid were added immediately before coating by a static mixer, so as to obtain a coating composition for a surface protective layer, which was transported to a coating die to make 8.3 mL/m<sup>2</sup>.

The coating composition had a viscosity measured with a B-type viscometer of Tokyo Keiki of 19 mPa·s at 40° C. (No. 1 rotor at 60 rpm).

(Preparation of Photothermographic Material 1)

On the back surface of the undercoated support, the antihalation layer coating composition to provide absorption of 0.3 at 504 nm and the back surface protective layer coating composition to provide a gelatin coated amount of 1.7 g/m<sup>2</sup> were simultaneously coated and dried to form a backing layer.

On the undercoating layer on the opposite side to the back surface, an emulsion layer, an intermediate layer, a first layer of a protective layer and a second layer of a protective layer were simultaneously coated in this order by the slide bead coating method to produce a sample of a photothermographic material. The temperatures of the emulsion layer and the intermediate layer were adjusted to 31° C., the temperature of the first layer of a protective layer was adjusted to 36° C., and the temperature of the second layer of a protective layer was adjusted to 37° C.

The coated amounts (in terms of g/m<sup>2</sup>) of the compounds in the emulsion layer were as follows.

|                                    |       |
|------------------------------------|-------|
| Silver behenate                    | 5.55  |
| Polyhalogen compound 1             | 0.02  |
| Polyhalogen compound 2             | 0.06  |
| Phthalazine compound 1             | 0.19  |
| SBR latex                          | 9.67  |
| Reducing agent 2                   | 0.81  |
| Hydrogen bonding compound 1        | 0.30  |
| Development accelerating agent 1   | 0.004 |
| Development accelerating agent 2   | 0.010 |
| Development accelerating agent 3   | 0.015 |
| Toning agent 1                     | 0.010 |
| Mercapto compound 2                | 0.002 |
| Silver halide (in terms of silver) | 0.091 |

The coating and drying conditions were as follows.

55 The coating was carried out at a rate of 160 m/min with a gap between the tip end of the coating die and the support of from 0.10 to 0.30 mm, and the pressure of the decompression chamber was set at a value lower than the atmospheric pressure by 196 to 882 Pa. The support was destinated with an ionic stream before coating.

60 The coating composition thus coated was cooled in the subsequent chilling zone with an air flow having a dry-bulb temperature of from 10 to 20° C., and the coated assembly was transported without contact and was dried in a helical non-contact dryer with a drying air flow having a dry-bulb temperature of from 23 to 45° C. and a wet-bulb temperature of from 15 to 21° C.

49

After drying, the assembly was adjusted for moisture content at 25° C. and 40 to 60% RH, and the film surface was heated to a temperature of from 70 to 90° C. After heating, the film surface was cooled to 25° C.

The thus produced photothermographic material had a matting degree in terms Beck's smoothness of 550 seconds on the photosensitive layer side and 130 seconds on the backing layer side. The measurement of the pH on the film surface on the photosensitive layer side revealed that it was 6.0.

The chemical structures of the compounds used in the example of the invention will be described below.



Tellurium sensitizer C



Blue Dye compound 1



Yellow dye compound 1



Reducing agent 2

50

-continued



Hydrogen bonding compound 1



Polyhalogen compound 1



Polyhalogen compound 2



Mercapto compound 2



Phthalazine compound 1



Development accelerating agent 1



Development accelerating agent 2



53

(Preparation of Silver Halide Emulsion 5)

A silver halide emulsion 5 was produced through the following steps.

A pure silver iodide emulsion A was produced in the same manner as in the silver halide emulsion 2 except that the solution A was a solution obtained by adding distilled water to 59.26 g of silver nitrate to make 520 mL, the total amount of which was added at a constant flow rate over 80 minutes, and the solution B was added by a CDJ method while maintaining pAg at 10.0.

1,420 mL of distilled water, the total amount of the pure silver iodide emulsion A thus prepared, 9.2 g of phthalated gelatin and 3.1 mL of a 1% by weight potassium bromide solution were mixed to form a solution, and the liquid temperature of the solution was maintained at 35° C. in a stainless steel reaction vessel. The total amount of a solution A, which was formed by diluting 14.8 g of silver nitrate with distilled water to make 260 mL, was added at a constant flow rate over 26 minutes, and a solution B, which was formed by diluting 12 g of potassium bromide with distilled water to make 300 mL, was added by a CDJ method while maintaining pAg at 10.0.

After terminating the stirring and subjecting to sedimentation, desalination and water washing steps, the pH was adjusted to 5.9 by using a sodium hydroxide solution having a concentration of 1 mole/L to produce a silver halide dispersion. A silver halide emulsion 5 was prepared in the same manner as in the production of the photothermographic material 1 with respect to the other conditions.

The particles in the silver halide emulsion thus prepared were silver iodobromide particles having an average sphere-equivalent diameter of 0.04  $\mu\text{m}$  and a variation coefficient of the sphere-equivalent diameter of 22%. They were silver halide particles, in which a silver iodobromide structure having an iodine content of 15% by mole was present through junction in the vicinity of the surface by a depth of about 4 nm from the particle surface.

A photothermographic material 9 was produced under the same conditions as in the production of the photothermographic material 1 except for the use of the silver halide emulsion 5. A photothermographic material 10 was produced under the same conditions as in the production of the photothermographic material 2 except for the use of the silver halide emulsion 5.

(Production of Photothermographic Materials 11 and 12)  
(Preparation of Silver Halide Emulsion 6)

1,420 mL of distilled water, 850 g of the silver halide emulsion 2, 9.2 g of phthalated gelatin and 3.1 mL of a 1% by weight potassium bromide solution were mixed to form a solution, and the liquid temperature of the solution was maintained at 35° C. in a stainless steel reaction vessel. The total amount of a solution A, which was formed by diluting 7.4 g of silver nitrate with distilled water to make 130 mL, was added at a constant flow rate over 13 minutes, and a solution B, which was formed by diluting 6 g of potassium bromide with distilled water to make 150 mL, was added by a CDJ method while maintaining pAg at 10.0.

After terminating the stirring and subjecting to sedimentation, desalination and water washing steps, the pH was adjusted to 5.9 by using a sodium hydroxide solution having a concentration of 1 mole/L to produce a silver halide dispersion. A silver halide emulsion 6 was prepared in the same manner as in the production of the photothermographic material 1 with respect to the other conditions.

54

The particles in the silver halide emulsion thus prepared were silver halide particles having an average sphere-equivalent diameter of 0.04  $\mu\text{m}$  and a variation coefficient of the sphere-equivalent diameter of 19%, in which a silver iodobromide structure having an iodine content of 25% by mole was present through junction in the vicinity of the surface by a depth of about 4 nm from the particle surface.

A photothermographic material 11 was produced under 10 the same conditions as in the production of the photothermographic material 1 except for the use of the silver halide emulsion 6. A photothermographic material 12 was produced under the same conditions as in the production of the photothermographic material 2 except for the use of the silver halide emulsion 6.

(Production of Photothermographic Materials 13 and 14)  
(Preparation of Silver Halide Emulsion 7)

A silver halide emulsion 7 was obtained in the same 20 manner as in the preparation of the silver halide emulsion 6 except that the solution B was added under the liquid temperature maintained at 50° C. by a CDJ method while maintaining the pAg at 9.4.

A photothermographic material 13 was produced under the same conditions as in the production of the photothermographic material 1 except for the use of the silver halide emulsion 7. A photo thermographic material 14 was produced under the same conditions as in the production of the photothermographic material 2 except for the use of the silver halide emulsion 7.

(Production of Photothermographic Materials 15 to 22)  
(Preparation of Silver Halide Emulsions 8 to 11)

Silver halide emulsions 8 to 11 having the compositions shown in Experiment Nos. 8 to 11 in the Table 1 were prepared in the same manner as in the preparation of the silver halide emulsion 5 except that the addition amounts of 35 the solutions A and B were changed.

The particles in the silver halide emulsion thus prepared were silver iodobromide particles having an average sphere-equivalent diameter of 0.04  $\mu\text{m}$  and a variation coefficient of the sphere-equivalent diameter of 18%. They were silver halide particles, in which a silver iodobromide structure having an iodine content shown in the Table 1 was present through junction. The silver iodobromide structure was present in the vicinity of the surface by a depth of about 50 nm from the particle surface.

Photothermographic materials 15, 17, 19 and 21 were produced under the same conditions as in the production of the photothermographic material 1 except for the use of the silver halide emulsions 8 to 11. Photothermographic materials 16, 18, 20 and 22 were produced under the same conditions as in the production of the photothermographic material 2 except for the use of the silver halide emulsions 8 to 11.

60 (Evaluation of Photothermographic Materials 1 to 22)

The photosensitive materials 1 to 22 obtained in the foregoing were evaluated in the following manner.  
(Exposure of Photosensitive Material)

65 The photosensitive materials obtained in Examples 1 to 8 were subjected to an exposure treatment in the following manner.

A semiconductor laser NLHV3000E produced by Nichia Corp. was installed in an exposure part of Dry Imager FM-DP L by Fuji Medical Systems Inc., and the beam diameter was narrowed down to about 100  $\mu\text{m}$ . Exposure of the photosensitive material was carried out for 10–6 second while the illuminance of laser light on the surface of the photosensitive material was changed from 0 and 1 to 1,000  $\text{mW/mm}^2$ . The light emission wavelength of the laser light was 405 nm.

(Development of Photosensitive Material)

The photosensitive materials thus exposed were subjected to a thermal development treatment in the following manner.

In the thermal developing part of Dry Imager FM-DP L by Fuji Medical Systems Inc., four plate heaters were set at 112°C, 115°C, 118°C and 121°C, respectively, thermal development was carried out to make a total thermal developing time of 14 seconds by increasing the film conveying speed.

(Evaluation of Samples)

The resulting images were measured for density by a densitometer, and a characteristic curve of densities with respect to logarithm of the exposure amount was prepared. An optical density on the non-exposed part was designated as fogging, and a reciprocal of the exposure amount providing an optical density of 3.0 was designated as sensitivity, which was expressed as a relative value with the sensitivity of the photosensitive material 3 being 100.

The results are shown in the Table 1.

5  
10  
15

materials of the invention have high sensitivities with small desensitization widths due to the polyhalogen in comparison to the comparative examples.

5  
10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880  
8885  
8890  
8895  
8900  
8905  
8910  
8915  
8920  
8925  
8930  
8935  
8940  
8945  
8950  
8955  
8960  
8965  
8970  
8975  
8980  
8985  
8990  
8995  
9000  
900

TABLE 2

| Experi-<br>ment<br>No. | Photo-<br>sen-<br>sitive<br>material | Wavelength<br>of exposure<br>laser (nm) | Total silver<br>iodide<br>content<br>(% by mole) | Total silver<br>bromide<br>content<br>(% by mole) | Ratio of silver<br>iodide/silver<br>bromide in junction<br>part of silver<br>iodobromide | Content<br>of junction<br>part (%<br>by mole) | Phthalazine<br>compound<br>(mole/<br>Ag mole) | Sensitivity to polyhalogen amount |                           |                     |
|------------------------|--------------------------------------|-----------------------------------------|--------------------------------------------------|---------------------------------------------------|------------------------------------------------------------------------------------------|-----------------------------------------------|-----------------------------------------------|-----------------------------------|---------------------------|---------------------|
|                        |                                      |                                         |                                                  |                                                   |                                                                                          |                                               |                                               | Polyhalogen<br>amount (1)         | Polyhalogen<br>amount (2) | (1)/<br>(2)<br>Note |
| 10                     | 23, 24                               | 405                                     | 3.5                                              | 96.5                                              | —                                                                                        | 0                                             | 0.13                                          | 15                                | 7                         | 2.14 Comparison     |
| 11                     | 25, 26                               | 405                                     | 3.5                                              | 96.5                                              | —                                                                                        | 0                                             | 0.25                                          | 18                                | 10                        | 1.8 Comparison      |
| 12                     | 27, 28                               | 405                                     | 3.5                                              | 96.5                                              | —                                                                                        | 0                                             | 0.64                                          | 22                                | 12                        | 1.83 Comparison     |
| 13                     | 1, 2                                 | 405                                     | 3.5                                              | 96.5                                              | —                                                                                        | 0                                             | 1.27                                          | 24                                | 14                        | 1.71 Comparison     |
| 14                     | 29, 30                               | 405                                     | 3.5                                              | 96.5                                              | —                                                                                        | 0                                             | 6.35                                          | 27                                | 15                        | 1.8 Comparison      |
| 15                     | 31, 32                               | 405                                     | 95                                               | 5                                                 | 15/85                                                                                    | 4                                             | 0.13                                          | 78                                | 41                        | 1.90 Invention      |
| 16                     | 33, 34                               | 405                                     | 95                                               | 5                                                 | 15/85                                                                                    | 4                                             | 0.25                                          | 89                                | 51                        | 1.75 Invention      |
| 17                     | 35, 36                               | 405                                     | 95                                               | 5                                                 | 15/85                                                                                    | 4                                             | 0.64                                          | 94                                | 54                        | 1.74 Invention      |
| 18                     | 17, 18                               | 405                                     | 95                                               | 5                                                 | 15/85                                                                                    | 4                                             | 1.27                                          | 100                               | 60                        | 1.67 Invention      |
| 19                     | 27, 38                               | 405                                     | 95                                               | 5                                                 | 15/85                                                                                    | 4                                             | 6.35                                          | 105                               | 67                        | 1.57 Invention      |

It is clear from the Table 2 that in the case of the high silver iodide emulsion having a silver iodide junction part, the desensitization width due to the polyhalogen amount is decreased by increasing the coated amount of the phthalazine compound with respect to the silver halide.

### Example 3

(Evaluation under Low Illuminance of Photothermographic Materials 1 to 4, 9, 10, 13, 14, 17, 18, 21 and 22)

The photosensitive material of the invention exhibits high sensitivity with favorable characteristics particularly upon exposure at high illuminance for a short period of time.

The photosensitive material was subjected to exposure in the same manner as in Example 1 except that 1 KW tungsten light with an interference filter of 405 nm inserted. The illuminance was significantly weakened to 0 and from 0.001 to 0.1 mW/m<sup>2</sup> with a step wedge in comparison to the exposure in Example 1, and therefore, a necessary optical density was obtained to adjust the exposure time. The sensitivity was expressed as a relative value with the sensitivity of the photo sensitive material 3 being 100.

The results are shown in the Table 3 below.

TABLE 3

| Experi-<br>ment<br>No. | Photo-<br>sen-<br>sitive<br>material | Wavelength<br>of exposure<br>laser (nm) | Total silver<br>iodide<br>content<br>(% by mole) | Total silver<br>bromide<br>content<br>(% by mole) | Ratio of silver<br>iodide/silver<br>bromide in junction<br>part of silver<br>iodobromide | Content<br>of junction<br>part (%<br>by mole) | Phthalazine<br>compound<br>(mole/<br>Ag mole) | Sensitivity to polyhalogen amount |                           |                     |
|------------------------|--------------------------------------|-----------------------------------------|--------------------------------------------------|---------------------------------------------------|------------------------------------------------------------------------------------------|-----------------------------------------------|-----------------------------------------------|-----------------------------------|---------------------------|---------------------|
|                        |                                      |                                         |                                                  |                                                   |                                                                                          |                                               |                                               | Polyhalogen<br>amount (1)         | Polyhalogen<br>amount (2) | (1)/<br>(2)<br>Note |
| 20                     | 1, 2                                 | 405                                     | 3.5                                              | 96.5                                              | —                                                                                        | 0                                             | 1.27                                          | 610                               | 332                       | 1.84 Comparison     |
| 25                     | 3, 4                                 | 405                                     | 100                                              | 0                                                 | —                                                                                        | 0                                             | 1.27                                          | 100                               | 46                        | 2.17 Comparison     |
| 21                     | 9, 10                                | 405                                     | 80                                               | 20                                                | 15/85                                                                                    | 17.1                                          | 1.27                                          | 107                               | 56                        | 1.91 Invention      |
| 22                     | 13, 14                               | 405                                     | 90                                               | 10                                                | 15/85                                                                                    | 8                                             | 1.27                                          | 114                               | 61                        | 1.86 Invention      |
| 23                     | 17, 18                               | 405                                     | 95                                               | 5                                                 | 15/85                                                                                    | 4                                             | 1.27                                          | 115                               | 61                        | 1.89 Invention      |
| 25                     | 21, 22                               | 405                                     | 98                                               | 2                                                 | 15/85                                                                                    | 2                                             | 1.27                                          | 112                               | 57                        | 1.96 Invention      |

59

It is clear from the Tables 1 and 3 that the photosensitive materials of the invention exert high sensitivity in the case where they are exposed with high illuminance light in comparison to the case where they are exposed with low illuminance light. It is understood, however, that the tendency of the desensitization width due to the polyhalogen is reproduced under the low illuminance.

## Example 4

The evaluations were carried out in the same manner as in Example 1 except that laser light having a light emission wavelength of 395 nm. The photosensitive materials of the invention provided the same favorable results.

According to the invention, an excellent photothermographic material having high sensitivity with a small desensitization width due to the polyhalogen amount can be provided even though it is a silver halide photosensitive material having a high silver iodide content, and a process for forming an image using the same can also be provided.

This application is based on Japanese Patent application JP 2002-122270, filed Apr. 24, 2002, the entire content of which is hereby incorporated by reference, the same as if set forth at length.

What is claimed is:

1. A photothermographic material comprising:  
a support; and  
a photosensitive silver halide, a nonphotosensitive organic silver salt, a reducing agent, an organic polyhalogen compound and a binder,  
wherein the photosensitive silver halide comprises 90% by mole or more of a silver iodide and has a silver iodobromide structure having an average silver iodide content of 35% by mole or less in vicinity of a surface thereof.

2. The photothermographic material according to claim 1, which further comprises a compound represented by the following formula (1) in an amount of 0.2 mole or more per 1 mole of the photosensitive silver halide in a same side as the photosensitive silver halide, the side being defined by the support:

(1)



wherein R¹ and R² each independently represents a hydrogen atom or a group that can be substituted on a benzene ring.

3. The photothermographic material according to claim 2, wherein the amount of the compound represented by the formula (1) is 0.5 mole or more per 1 mole of the photosensitive silver halide.

4. The photothermographic material according to claim 2, wherein the amount of the compound represented by the

60

formula (1) is 1.0 mole or more per 1 mole of the photosensitive silver halide.

5. The phototherinographic material according to claim 1, wherein the photosensitive silver halide is formed under a state where the nonphotosensitive organic silver salt is not present.

6. The photothermographic material according to claim 2, wherein the photosensitive silver halide is formed under a state where the nonphotosensitive organic silver salt is not present.

7. The photothermographic material according to claim 3, wherein the photosensitive silver halide is formed under a state where the nonphotosensitive organic silver salt is not present.

8. The photothermographic material according to claim 1, wherein the average silver iodide content of the silver iodobromide structure in the vicinit of the surface is 25% by mole or less.

20 9. The photothermographic material according to claim 1, wherein the average silver iodide content of the silver iodobromide structure in the vicinity of the surface is 15% by mole or less.

10 10. The photothermographic material according to claim 1, which further comprises a compound represented by the following formula (D):



35 wherein R²¹ to R²³ each independently represents an alkyl group, an aryl group, an alkoxy group, an aryloxy group, an amino group or a heterocyclic group, which may be unsubstituted or substituted.

11. The photothermographic material according to claim 10, which comprises the compound represented by the formula (D) in an amount of from 1 to 200% by mole based on the reducing agent.

40 12. A process for forming an image comprising a step of exposing the photothermographic material according to claim 1 by a laser having a light emission peak at a wavelength of from 350 to 450 nm.

13. The process according to claim 12, wherein the laser has a light emission peak at a wavelength of from 390 to 430 nm.

50 14. The process according to claim 12, wherein the laser has an exposure illuminance of 1 mW/mm² more and an exposure time of 1 second or less.

15. The process according to claim 14, wherein the exposure time is 10⁻² second or less.

\* \* \* \* \*